

Feb. 14, 1961

F. E. RATH

2,971,703

PROCESS FOR CLEANING AND RECOVERING SCRAP  
METAL FROM SLAG AND THE LIKE

Filed June 4, 1958

13 Sheets-Sheet 1

FIG. 1a  
(PRE-PROCESSING)



Feb. 14, 1961

F. E. RATH

2,971,703

**F. E. RATH**  
PROCESS FOR CLEANING AND RECOVERING SCRAP  
METAL FROM SLAG AND THE LIKE

Filed June 4, 1958

13 Sheets-Sheet 2



Feb. 14, 1961

F. E. RATH

2,971,703

**P. E. RATH**  
**PROCESS FOR CLEANING AND RECOVERING SCRAP**  
**METAL FROM SLAG AND THE LIKE**

Filed June 4, 1958

13 Sheets-Sheet 3

**FIG. 1c**  
*(MAGNETIC SEPARATION  
AND REFINING)*



Feb. 14, 1961

F. E. RATH

2,971,703

T. E. RATH

PROCESS FOR CLEANING AND RECOVERING SCRAP  
METAL FROM SLAG AND THE LIKE

Filed June 4, 1958

13 Sheets-Sheet 4



INVENTOR:

INVENTOR.  
*FRANK E. RATH*

BY:

By:  
Green, McCallister & Miller

*HIS ATTORNEYS*

Feb. 14, 1961

F. E. RATH

2,971,703

PROCESS FOR CLEANING AND RECOVERING SCRAP  
METAL FROM SLAG AND THE LIKE

Filed June 4, 1958

13 Sheets-Sheet 5

FIG. 4



INVENTOR:  
FRANK E. RATH

BY:  
Green, McCallister & Miller

HIS ATTORNEYS.

Feb. 14, 1961

F. E. RATH  
PROCESS FOR CLEANING AND RECOVERING SCRAP  
METAL FROM SLAG AND THE LIKE

2,971,703

Filed June 4, 1958

13 Sheets-Sheet 6

**FIG. 4A**



**FIG. 5**



INVENTOR:  
**FRANK E. RATH**  
BY:  
*Green, McCallister & Miller*  
HIS ATTORNEYS.

Feb. 14, 1961

F. E. RATH

2,971,703

PROCESS FOR CLEANING AND RECOVERING SCRAP  
METAL FROM SLAG AND THE LIKE

Filed June 4, 1958

13 Sheets-Sheet 7



INVENTOR:  
**FRANK E. RATH**

BY:  
*Green, McCallister & Miller*

HIS ATTORNEYS.

Feb. 14, 1961

F. E. RATH

2,971,703

PROCESS FOR CLEANING AND RECOVERING SCRAP  
METAL FROM SLAG AND THE LIKE

Filed June 4, 1958

13 Sheets-Sheet 8

**FIG. 6A**



**FIG. 6B**

INVENTOR:

**FRANK E. RATH**

BY:

*Green, McCallister & Miller*

HIS ATTORNEYS.

Feb. 14, 1961

F. E. RATH

2,971,703

PROCESS FOR CLEANING AND RECOVERING SCRAP  
METAL FROM SLAG AND THE LIKE

Filed June 4, 1958

13 Sheets-Sheet 9

*FIG. 7*



*FIG. 8*



Feb. 14, 1961

F. E. RATH

2,971,703

PROCESS FOR CLEANING AND RECOVERING SCRAP  
METAL FROM SLAG AND THE LIKE

Filed June 4, 1958

13 Sheets-Sheet 10



INVENTOR:  
FRANK E. RATH  
BY:  
*Green, McCallister & Miller*  
HIS ATTORNEYS.

Feb. 14, 1961

F. E. RATH

2,971,703

Filed June 4, 1958

**F. E. RATH**  
PROCESS FOR CLEANING AND RECOVERING SCRAP  
METAL FROM SLAG AND THE LIKE

13 Sheets-Sheet 11



Feb. 14, 1961

F. E. RATH

2,971,703

Filed June 4, 1958

**F. E. RATH**  
**PROCESS FOR CLEANING AND RECOVERING SCRAP**  
**METAL FROM SLAG AND THE LIKE**

13 Sheets-Sheet 12

**FIG. 12**  
*(MAGNETIC SEPARATION AND REFINING  
 OF MINUS 3" MAGNETICS)*



Feb. 14, 1961

F. E. RATH

2,971,703

PROCESS FOR CLEANING AND RECOVERING SCRAP  
METAL FROM SLAG AND THE LIKE

Filed June 4, 1958



2,971,703

**PROCESS FOR CLEANING AND RECOVERING SCRAP METAL FROM SLAG AND THE LIKE**

Frank E. Rath, 724 E. Brady St., Butler, Pa.

Filed June 4, 1958, Ser. No. 739,823

16 Claims. (Cl. 241—24)

This invention relates to the selective recovery of materials from metal bearing refuse and debris, and particularly from slags, which are produced by steel plants in connection with the operation of steel producing units, such as basic open hearth, duplex, Thomas, Bessemer, oxygen blow or electric steel melting and refining furnaces or converters. It deals with the recovery of both magnetic and non-magnetic metals and high iron content magnetic materials from open hearth flush or runoff slags, open hearth tap or finishing slags, electric furnace or other steel producing slags, as well as from soaking pit bottom materials, rolling mill debris, or mixtures of all of these materials.

This application is a continuation-in-part of my co-pending application, Serial No. 674,255 of July 25, 1957, now forfeited, which is a continuation of my now-abandoned application, Serial No. 379,009 of September 8, 1953 of the same title.

The procedure is effected in such a manner that, for the first time, a substantially complete recovery of the magnetic and non-magnetic metals, and magnetic metal oxide content is accomplished. The materials thus recovered are separated, concentrated, and produced in such a clean and uncontaminated condition as to enable their re-use in the steel plant at a location where their maximum economic value is realized.

Thus, an important phase of my invention deals with the progressive and selective recovery and separation of valuable materials (value content) from steel plant slags and other refuse materials, based upon the size range and physical nature of the materials being processed, upon their malleable as distinguished from friable nature, and upon their magnetic and non-magnetic properties.

The near-exhaustion of the relatively pure, high grade iron ores of the Hibbing range in Minnesota, the scarcity of new, large domestic ore bodies, and the increasing cost and national defense factors of scarcity, shipping distance, screening, concentration, etc., of both foreign and domestic iron ores have all made the recovery of the valuable metal and metal oxide content of slags and steel plant debris an important matter economically, and also from the standpoint of national defense and the conservation of natural resources.

Heretofore, recovery of valuable materials from slags and steel plant refuse has been limited to attempts at recovery of magnetic metals. In the steel plants this is accomplished by a simple magnetic separation in the pouring pits and cinder yards of the steel producing unit, wherein the larger pieces of solid metal (generally in excess of 12 inches) are removed and after rough cleaning at a ball-drop are remelted in the steel producing unit or used as charge material in a blast furnace. Any incidental recovery of smaller magnetic materials is (because of contamination) almost invariably directed to the blast furnaces for re-use. In recent years a more intensive effort has been made to recover additional metallics at the waste refuse dumps of the steel plants, after most of the relatively large pieces of scrap metal

have been removed in the steel plant. Such metallics as are currently recovered at the slag dumps contain pieces of magnetic metal badly contaminated with slag, as well as quantities of magnetic open hearth slag and other impurities which limit the re-use of these metallics to the blast furnaces except for a limited amount of large metal pieces. In many instances these recovered metallics are so badly contaminated that material below say 1 inch in size must be screened out and discarded in order that the remaining material be acceptable in quality even for re-use in a blast furnace.

Inasmuch as a blast furnace is a preliminary smelting and reducing unit which provides metallic iron in a molten or solidified condition (pig iron) to the open hearth furnaces for refining and final production of steel ingots; it should be noted that, in addition to the loss of metallics which occurs in present processes (by a limited recovery of the metallics present in the refuse and by discarding under-size material), there is a further economic loss due to the necessity of re-using this material (because of contamination) in a blast furnace rather than by remelting it in an open hearth or other steel producing unit.

There is no process available today which enables substantially complete recovery of the valuable materials present in steel plant slags and refuse or which provides products of satisfactory quality. For example, no method is currently available which enables recovery of non-magnetic metal, or separation of magnetic metals and magnetic slags, except by hand picking or sorting. Few if any, of the procedures used today produce ordinary steel scrap in sizes below 12 inches clean enough to justify re-use of this metal in an open hearth or other steel producing unit, or is there any method available which controls the contamination in metallics prepared for blast furnace use.

My investigations have shown that a large amount of the material discarded in present processes as non-magnetic contains an appreciable quantity of valuable metal which is enclosed, bound, or carried by non-magnetic slag or cinder pieces, and which from an economic standpoint, should not be wasted. In this connection, particularly with regard to open hearth flush or runoff slag, various sized pieces of magnetic metal may be carried within a piece of flush or runoff slag and because of their location and embedded or bound relationship, or the relatively smaller proportionate size of the magnetic metal piece in comparison with the size of the non-magnetic matrix or embedding material, cannot be picked up by ordinary magnetic separation means such as an electromagnet. Open hearth tap slags containing substantial quantities of re-usable magnetic iron oxides are also lost in a similar fashion. The possibilities of recovery from this standpoint are tremendous and, as I have determined, actually predominate as to the recovery that may be effected from steel plant slags or debris.

Steel plant slags and debris, such as are here being considered, will consist primarily of basic open hearth slags. Basic open hearth slags consist essentially of two types of slag: (1) flush or runoff slag, and (2) tap or finishing slag. The flush or runoff slag is a tough, porous, essentially non-magnetic slag with a high phosphorous content containing pieces of entrapped steel, varying in size from  $\frac{1}{8}$  of an inch and smaller up to 6 and 8 inches or larger. By contrast, tap or finishing slag is a rather friable, dense slag with a relatively low phosphorous content which varies in iron content and magnetic characteristics from moderately magnetic to very highly magnetic and with no entrapped metal particles as such. Also, I have discovered small fragments within a given piece of tap slag will vary widely as to their iron and phosphorous content and magnetic characteristics. In

addition to these two slags as such, there will also be pouring side cleanup material from the open hearth, consisting of mixtures of both types of slags plus steel spills that occur in the course of furnace tapping, ingot teeming, and slag runoffs. An incidental amount of refractory brick will also be encountered in this cleanup material from ladle and furnace linings.

Depending on the particular steel plant, Bessemer, Thomas, Oxygen Blow, and Duplex furnace or converter slags may also be encountered together with slags and bottom material from soaking pits and reheating furnaces, and refractory materials from furnace rebuilds, all of which contain steel and magnetic iron oxides. The other types of steel producing slags and debris are similar to open hearth slags except that pouring pit cleanup from an electric furnace plant may include a certain amount of non-magnetic stainless steel scrap.

The steel producing slags and other steel plant debris as described have little value for any known purpose, except for use as fill material, but certain of the components have a very definite economic value if they can be properly separated and cleaned.

The total economic value of the various constituents depends not only on the separation of the valuable constituents of the mixture from undesirable contaminants but also on the completeness of their separation from one another. For example, stainless steel scrap has a very high value for melting in an electric furnace to produce stainless steel, but if this scrap is mixed with ordinary steel scrap its value is reduced to the value of the ordinary scrap. In the same fashion, ordinary steel scrap, clean and free of slags and other contaminants, has a high value for remelting in an open hearth furnace to produce steel ingots. If, however, this steel scrap is contaminated with adhering flush slags, magnetic tap slags and other metal oxides, the scrap in the resultant mixture, which is of little use in an open hearth, has a much lower value as blast furnace charge material. Similarly, small particles of metal, roll scale and high iron content tap slags when properly sized, and if low in phosphorous contamination, constitute an excellent iron bearing material for blast furnace use which is superior to the highest grade iron ores. Again, if these iron bearing materials are diluted with flush slag so that the iron content is reduced and the phosphorous contamination becomes unduly high, they are not usable to any extent even as a low grade blast furnace charge. There is thus an important economic need in the steel industry for a process which can be used on all types of metal bearing refuse and debris to recover and separate the various valuable components in these materials. Such a process, to be of maximum value, should (1) recover all of the valuable components free of undesirable materials and contamination, and (2) should separate and segregate these materials so that each recovered component is suitable for use in a process where its greatest economic value can be realized.

There is no process or method of recovery available to the steel industry which satisfies either of these requirements.

It has thus been an object of my invention to devise a process which will practically and economically satisfy these requirements and which will eliminate the rough, makeshift, wasteful, and superficial approaches that have heretofore been made in processing steel plant slags and metal bearing debris;

Another object has been to develop an economical, efficient, and substantially continuous processing procedure or system for the complete recovery, separation, and segregation of the value content of steel plant slags and other debris, which can be installed at or near a steel plant cinder yard and operated in a continuous manner with a minimum cost of operation and maintenance for the apparatus involved, and which will enable direct processing of steel plant slags from the cinder yard, after a

pick-out removal of obvious, large pieces of metal in the yard, and which will provide for collecting the recovered materials in such a manner as to make possible their most advantageous and economic employment;

5 Another object has been to devise a new and improved procedure or system for progressively and selectively recovering substantially all of the metal content of steel plant slags and metal bearing debris, whether such metal is magnetic or non-magnetic and for completely separating and segregating these metals from each other and 10 from other materials, including magnetic slags and magnetic iron oxides, so that such recovered metals may be re-used, to the extent that their physical size permits, directly in an open hearth or electric steel melting furnace;

15 Another object has been to develop a process or procedure which will enable recovery of all or substantially all of the smaller steel particles which are embedded in open hearth flush slags and other steel plant slags and debris, and to clean and purify these recovered metal particles without loss or size reduction;

20 A further object of my invention has been to develop a process which will recover and concentrate high iron and low phosphorous content magnetic tap slags and iron oxides and reject low iron and high phosphorous content magnetic tap slags and magnetic iron oxides without reducing the particle size of the majority of the product below a practical limit for direct blast furnace use;

25 A further object of my invention has been to take a process mixture of materials of many characteristics, sizes and nature, and while moving them as a stream, to progressively and selectively sort them out in such a manner that a substantially complete recovery of the metal or metal-bearing content may be effected;

30 These and other objects of my invention will appear to those skilled in the art from the layout drawings, illustrated apparatus, and the description thereof;

35 Figures 1a, 1b, and 1c are somewhat diagrammatic broken plan views which, when taken together, illustrate 40 a layout or an arrangement of facilities for a complete process or system to be constructed and employed in accordance with my invention;

45 Figure 1a represents the preliminary or pre-processing portion of the illustrated embodiment of a processing system employed in accordance with my invention; Figure 1b represents the intermediate portion of metal cleaning and separation, and Figure 1c represents the final portion of the same system wherein magnetic separation, refining and concentration is effected.

50 It will be noted that Figure 1a is to be placed adjacent to Figure 1b along line X—X and that Figure 1b is, in turn, to be placed adjacent to Figure 1c along line XX—XX to provide the complete, continuous system.

55 Figure 2 is a side section in elevation, somewhat diagrammatically illustrating a dump truck discharging slag materials for processing upon a roller type screening device which, in turn, is discharging oversize materials upon a steel apron-type conveyor, with the undersize materials falling through the roller screen into a storage bin or hopper; also shown in dotted outline immediately above the roller screen is a clamshell bucket which may be employed either with a crawler-mounted boom crane of conventional design or with an electric, overhead traveling crane on a runway; either the truck, the bucket or both 60 provide for charging materials upon the roller screen; this view is taken along line II—II of Figure 1a (see the lower left hand corner);

65 Figure 3 is a side section in elevation showing the lower portion of the hopper of Figure 2, together with an electric vibrating feeder to discharge material out of the hopper upon a belt type conveyor; this view is taken along line III—III of station A of Figure 1a;

70 Figure 4 is a side section in elevation showing a rotary crusher or impactor constructed and employed in accordance with my invention, with oversize slag material from

the apron conveyor of Figure 2 entering the impactor and after impacting, being discharged upon a belt type conveyor; this view is taken along the line IV—IV of station B of Figure 1a;

Figure 4A is an end section in elevation of the same scale as and taken along line IVA—IVA of Figure 4;

Figure 5 is a fragmental side section in elevation showing a belt conveyor feed to an impactor apparatus such as disclosed in Figure 4 and is taken along the line V—V of Figure 1b;

Figure 6 is an enlarged side section in elevation of a roller screen device for employment in accordance with my invention along the line VI—VI of station E of Figure 1b;

Figure 6A is an enlarged plan view of this roller screen;

Figure 6B is a somewhat fragmental side view in elevation taken along the line VIB—VIB of Figure 6A;

Figure 7 is a somewhat diagrammatic side section in elevation of a magnetic pulley with conveyor belt to separate magnetic and non-magnetic clean metal, and to discharge the separated metals upon receiving belt conveyors; this view is taken along the line VII—VII of station F of Figure 1b;

Figure 8 is a side view in elevation of a self-cleaning, cross-belt, rectangular magnet employed in accordance with my invention, and showing pick-up and discharge of magnetic materials; this view is taken along line VIII—VIII of station M of Figure 1c but discharge chute 83 of Figure 8 has been omitted in Figure 1c;

Figure 9 is a side view in elevation, partially sectioned, showing the removal of magnetics by the cross-belt rectangular magnet of Figure 8 and by a magnetic pulley, with magnetic materials from both being combined and discharged upon a belt conveyor; non-magnetic residue is also shown being discharged from the belt conveyor upon a vibrating screen, with undersize non-magnetics passing through the screen upon a conveyor and oversize material going across the screen into a roll-type crusher and then to a belt conveyor; this view is taken along line IX—IX of stations M, N and O of Figure 1c;

Figure 10 is a side sectional view in elevation of a belt conveyor discharging magnetic materials upon a vibrating screen, with undersize materials passing through the screen upon a belt conveyor, and oversize magnetic materials going across the screen and into a magnetic separator; also shown is product discharge at the far right out of the separator onto a belt conveyor, with the rejects from the separator chuted into a roll-type crusher, and then onto a belt conveyor; this view is taken along line X—X of stations P and Q of Figure 1c;

Figure 11 is a somewhat larger side sectional view of a magnetic separator, showing magnetic fines being fed into the separator, and the product at the far right and rejected magnetic fines being discharged upon belt conveyors; this view is taken along line XI—XI of station T of Figure 1c;

Figure 12 is a somewhat diagrammatic broken plan view which, when placed along line Z—Z of Figure 1b and as combined with Figure 1a, illustrates another complete, continuous system which employs principles and facilities of my invention to meet an exemplary set of steel plant requirements;

Figure 13 is a somewhat diagrammatic plan view illustrating a complete, continuous system employing principles and facilities of my invention in a further cooperative functional relationship to meet another exemplary set of plant requirements as to product size, nature and content.

#### General process considerations and procedures

Practically all steel plants, in the normal course of sorting and loading out their waste steel producing slags and other metal bearing debris, retrieve the large, obvious pieces of scrap metal before wasting this material. The

scrap thus recovered, is generally above 12 inches in size and includes steel skulls and "buttons" some of which are as large as eight to ten feet in diameter and weigh many thousands of pounds. This scrap is normally transferred to a skull cracker or ball drop and is cleaned by ball dropping and then cut as required into smaller sizes for recharging into the furnaces. In general my process contemplates the processing of steel producing slags and debris after the larger pieces of scrap metal (over 12 inches) are recovered by this preliminary sorting-out action in the steel plant cinder yards.

The primary problem in processing the residual slag materials at this stage, is that of releasing, cleaning, and separating the metal content of the mixture (both magnetic and non-magnetic) from the various slags and other contaminating materials. The larger pieces of metal (above 1 inch in size) are very acceptable for open hearth or electric furnace use while the smaller particles of metal (because of size) are more acceptable for blast furnace use.

The slags and other materials in this mixture vary in piece size from approximately 24 inches down to dust, and will contain rough, irregular pieces of metal from 12 inches mesh size down to less than  $\frac{1}{100}$  of an inch mesh size. The metal content, as previously mentioned, is generally not free but is rather embedded in a matrix of tough, abrasive, non-magnetic slag or other foreign material. In addition, it should be noted that both magnetic and non-magnetic slags are present in the mixture.

A secondary problem in completely processing this material is that of selectively recovering, cleaning, and concentrating those portions of the magnetic slags and magnetic oxides present in the mixture which I have discovered have a high enough iron content and a low enough phosphorous content to warrant their re-use in a blast furnace for iron production. Desirably, a maximum amount of these magnetic slags, when recovered, should be of such size (above  $\frac{1}{4}$  of an inch) that direct re-use in a blast furnace can be effected without the necessity of agglomerating procedures.

Reference to Figures 1a, 1b and 1c will indicate that my system or procedure is divided into three principal parts. This division is based upon practical considerations discovered in developing my invention, and as applied to the size and nature of the material being handled and processed. In what I designate as a pre-processing part of the procedure (see Figure 1a), I, in effect, provide a process burden consisting of slags, metals, etc., all of which has been broken down to an indicated minus 12 inch grid or screen mesh size, ready for an important second part of my procedure.

In the second part (see Figure 1b), the metal content of a size suitable for direct charging into open hearth and electric furnaces is released, cleaned, and separated out with respect to the remainder of the burden. Simultaneously, the average piece size of the burden is reduced and smaller metal pieces and desirable magnetics are released from the slag and the other foreign material in which they were embedded. It should be noted that screening devices are used at each stage to bypass the smaller size material. This is done so that only material of a size range suited to the operating characteristics of each impactor will be fed at a particular station and thus avoid useless wear of the impacting means. In addition, this by-pass arrangement avoids excessive size reduction of magnetics which are to be recovered at a subsequent stage of the process.

The cleaning and separating of the metal content of the burden is effected by a new and improved type of apparatus, in the nature of rotary impact crushers, devised and constructed in accordance with my invention, and effectively used with roller screens and electric vibrating screens for separating metal content down to 1 inch mesh size. The metals themselves, being malleable, are not broken up by my type of impacting-crushing ac-

tion, while the other constituents of the process burden, including magnetic and non-magnetic slags, are.

In the third and final part of my procedure or system (see Figure 1c), the burden or material of an indicated minus 1 inch size range is effectively separated into magnetic and non-magnetic portions and the separate portions successively and progressively processed down to substantially its full extent for recovery of the value content of the burden.

10 Electrically vibrated screens are used to separate the magnetic materials into specific size classifications to enable the purification and refining procedures which follow. Roll crushers are used in releasing or breaking away and segregating-out the magnetic metal and desirable magnetic slag content in combination with magnetic selectors or separators. The procedures employed in this part of my process provide clean metal particles as well as a high quality magnetic slag material in an indicated size range of  $\frac{1}{8}$  to minus 1 inch which is shown delivered to collecting area (5) for direct utilization in a blast furnace, for example. Smaller metal and desirable magnetics, in a size range from minus  $\frac{1}{8}$  of an inch to dust, are shown delivered to a collecting area (6) from which point they may be delivered to a sintering or agglomerating unit for more advantageous employment in, for example, a blast furnace.

On the other hand, non-magnetic slag material under minus  $\frac{3}{8}$  of an inch mesh size together with rejected magnetic material under  $\frac{1}{8}$  of an inch mesh size, is delivered to collecting area (4) for such use as may be advisable. As a result, my system effects a substantially complete recovery, segregation, and separating out of the value content of the original process burden, and does it automatically by apparatus in such combination that efficient and effective operations are accomplished throughout, continuously. It is done in such a manner and by apparatus that has a low upkeep cost, even under severe conditions and heavy utilization. In other words, the nature and utilization of each piece of apparatus, as well as its location is such that the most effective and economical recovery of the value content is accomplished for most efficient product utilization, with a minimum of wear and tear on the apparatus. In general, the apparatus is all employed in a fully coordinated and cooperative manner of functioning in accordance with my invention.

In detail, my procedure, consists of breaking oversize slag pieces in the pre-process area of Figure 1a, and thereafter involves a continuous line type of operation, as illustrated in Figures 1a, 1b, and 1c, wherein a process mixture of a maximum size content of approximately 12 inches, which I have determined is practical for handling, on present day rubber conveyor belts, is continuously moved, while it is subjected to progressive station operations. The station operations importantly include an impact crushing of the more or less friable slag materials to release valuable metals and metal oxides and a simultaneous impact cleaning of larger metal pieces to free them from slag contamination. Apparatus, such as represented by Figures 4 and 5 of the drawings, is especially designed and constructed to meet the peculiar needs of my concept in this connection.

Those approximate rotor speeds which have been found to be effective for each of the various size ranges of material being processed are shown on Figures 1a and 1b in terms of feet per minute speed at the impact blade tip, and for a particular diameter rotor, in terms of revolutions per minute.

It is highly important to free the magnetic metals and magnetic oxide materials from each other and from the binding material or materials, so that a full and maximum recovery may be effected. The handling of the process materials within the impacting apparatus, as well as the construction of such apparatus, has to be such that the apparatus will have a good period of useful life without

5 breakdowns and costly repairs. These and other factors enter into providing impactors at each impacting or breaking-up station that have a proper piece size range of materials being fed a proper speed of rotor or impeller means, and a proper size of opening or throat through which the materials enter and are discharged. The operation must be progressive and selective in order to obtain a substantially full and economic recovery of clean, uncontaminated metal.

10 The freed metal pieces which are essentially non-breakable or non-friable from the standpoint of my apparatus are, in accordance with my invention, recovered in progressively smaller size range stages on the basis of their relatively larger sizes or size range with 15 respect to selectively broken-up portions of the process material, and after all of the non-metal material has been broken-up into a size range below that of the selected size range of free metal that is to be taken off or selectively removed at a particular stage or station. 20 It may be noted that the volume of the burden is substantially the same throughout the processing except for the clean metal removed, but the size range of the burden becomes progressively smaller.

25 The metal content which is selectively recovered along my continuous processing line is shown divided into three size ranges that progressively decrease in size from about a 6 to 12 inch size range, to a 3 to 6 inch size range, and down to a minimum size range of about 1 to 3 inches, all of which are separated from the process mixture by screen type separating means. After separation 30 of the metal from the process mixtures, the various size ranges are combined as shown and the recovered clean metal is separated into magnetic and non-magnetic components by use of a magnetic pulley as shown in Figure 7.

35 The magnetic separation of clean metals at this point, enables a separation of ordinary steel scrap from non-magnetic stainless steels. Since non-magnetic stainless steel scrap has a high value for re-use in the electric furnaces, whereas ordinary or magnetic grades of steel scrap are generally re-used in an open hearth furnace, the metals recovered at this stage after separation are designated as to their point of re-use.

40 At this stage of the processing, impacting and screen separation are discontinued and the next stage of the processing namely; magnetic separation, refining, and concentration of the smaller metal particles, magnetic slags and oxides begins; since, (1) the maximum piece size of material in the process burden has been reduced to a size from which magnetic material may be effectively 45 separated by magnetic means, (2) little or no non-magnetic scrap occurs below this size range which necessitates this type of separation, (3) there is no further need to segregate magnetic metals, magnetic slags, and magnetic oxides below this size range, since all of the metal bearing material recovered, below 1 inch in size, is best suited for re-use in the blast furnace, and (4) in this 50 size range and particularly, after removal of larger non-crushable magnetic metals by magnetic means, roll crushers are suitable and more economical than impact breaking for any further size reduction that is desired 55 to free entrapped, recoverable materials.

60 Throughout this disclosure, when I speak of a size or size range, I have reference to a particular shape and size of the pieces or particles which will pass through a 65 specified screen mesh, guide or roll pass size or opening that has equal cross-dimensions (perpendicular to each other). Thus, I am not actually referring directly to the size of the shape, piece or particle, but indirectly to its size from the standpoint of the mesh or opening through which it will pass. This designation is believed to be the most accurate one, since the pieces, particles or shapes, are not essentially uniform from the standpoint of their configuration and may be in the nature of slivers and other odd shapes.

70 At this stage of the processing, at the left side of Figure

1c; since all of the components of the process mixture are under 1 inch maximum piece size, high intensity magnetic fields are effectively employed to separate the magnetic and non-magnetic portions of the process burden. After magnetic separation, there will still remain in the non-magnetic portion of the burden small magnetic metal particles (less than  $\frac{1}{4}$  of an inch) which are embedded in relatively large pieces ( $\frac{3}{4}$  to 1 inch) of non-magnetic slag or other non-magnetic material which do not respond to the magnetic fields. The high intensity magnetic fields are shown applied by two separate devices from two directions while the burden is moving on a rubber conveyor belt, with a preferred burden depth of approximately 1 inch. The burden depth is controlled by the width of belt employed and the speed of travel of the belt. The first magnetic device shown (Figure 8) is a self-cleaning rectangular electro-magnet suspended approximately 3 to 4 inches above the conveyor belt. This device removes most of the larger magnetic material and the smaller magnetic material in the upper portion of the process burden.

The second device shown (Figure 9) is a high intensity electromagnetic pulley 85 which operates as the drive pulley of the conveyor belt 27c and removes the balance of the magnetic material as the process burden is freely discharged across the face of the magnetic drive pulley. The crude magnetic materials removed by both of these devices are shown discharged and combined on a separate rubber belt conveyor 34. The non-magnetic portion of the process burden is shown discharged onto a  $\frac{3}{8}$  inch mesh electric vibrating screen O' from which material under  $\frac{3}{8}$  of an inch (which is essentially free of any recoverable metal content) is transferred on to another conveyor 33b for disposal. The non-magnetic process burden over  $\frac{3}{8}$  of an inch, is shown as fed into a roll crusher 160 with the rolls set to produce minus (—)  $\frac{3}{8}$  of an inch product which releases any small particles of free magnetic metal from the larger pieces of non-magnetic material. The material from the roll crusher is then shown as returned to the main process conveyor 27c by conveyors 35, 35a and 35b to be subjected again to the high intensity magnetic fields previously described.

The crude magnetics which were separated from the non-magnetic process burden are shown separated into three separate size ranges by vibrating screens P' and R', namely;  $\frac{3}{8}$  to 1 inch,  $\frac{1}{8}$  to  $\frac{3}{8}$  of an inch, and minus (—)  $\frac{1}{8}$  of an inch. Each size range is separately fed into a magnetic separator, such as shown in Figure 11. This type of separator consists of a self-cleaning electromagnet 99 with alternate north and south poles suspended above a non-magnetic conveyor feed belt 27f. By varying the D.C. current input to the electromagnet by means of a D.C. rheostat and adjusting the distance of the magnet and top conveyor belt from the process material, it is possible in this separator, when the feed material input is within a limited size range, to selectively separate relatively pure clean metal particles and high iron-low phosphorous content magnetic slags and magnetic oxides, on the one hand, from relatively impure, slag-contaminated metal particles and lower iron-higher phosphorous content magnetic slags and magnetic oxides; on the other. Thus it is possible to control the quality of product which will be discharged from the separator. The two classes of material, hereafter referred to as product and rejects, respectively, are shown in Figure 11 as separately discharged by chutes located below and slightly forward of the magnet bank into conveyor belts 37 and 33 respectively.

By roll crushing the rejects, Figure 10, from the two magnetic separators Q and S (Figure 1c), which operate on the larger size ranges of crude metallics, contaminated metal particles rejected in the larger size ranges are freed from adhering slag and are subsequently recovered by recycling without loss of metal or reduction of metal particle size. In similar fashion and simultaneously, the

pieces of magnetic slags and oxides with a high average iron content (and low phosphorous) which have the highest magnetic attraction will be discharged from the separators as product. The medium and lower iron content slags and oxides (and higher phosphorous content) of lesser magnetic attraction will be rejected. By crushing these rejected magnetic slags and oxides in the larger size ranges, the larger pieces are broken into smaller pieces which I have discovered will vary greatly in their iron and phosphorous content. By recycling this crushed material, those pieces with a high iron and low phosphorous content will be subsequently recovered in the smaller sized products. Although there is a size reduction of the magnetic slags which occurs in this procedure, the crushing is deliberately minimized and conducted by steps, as shown ( $\frac{3}{8}$ " pass roll crusher 87 at station Q and  $\frac{1}{8}$ " pass roll crusher at station S), in order to avoid unnecessary size reduction. Because of practical considerations relating to crushing costs and diminishing product value and yield, particle size reduction of rejects below  $\frac{1}{8}$  of an inch is not shown in the processing of crude metallics.

It should be noted that use of the magnetic separator, in itself, cannot economically accomplish the desired results in processing and refining crude metallics but must be used in a combination crushing and recycling arrangement as shown. Thus by the use of equipment and processing shown in Figures 1c, 8, 9, 10 and 11, substantially complete or maximum recovery, purification, and concentration of re-usable iron bearing magnetic materials is effected. Since metal bearing materials as small as  $\frac{1}{8}$  of an inch in size may be used in a blast furnace without excessive dust loss, the  $\frac{3}{8}$  to 1 inch, and  $\frac{1}{8}$  to  $\frac{3}{8}$  of an inch size range products from the magnetic separators 30 Q and S are shown combined into a single  $\frac{1}{8}$  to 1 inch product on conveyor 36 for direct blast furnace use. As shown in Figure 1c, magnetics below  $\frac{1}{8}$  of an inch in size are concentrated in a third magnetic separator at station T, Figure 11, and the product conveyed by conveyor 37 35 to a separate area. This product should preferably be agglomerated in a sinter plant (along with flue dust and ore fines) before attempting to use it in a blast furnace in order to avoid excessive dust loss in the furnace.

#### Process line apparatus

45 By way of example, and particularly referring to Figure 1a, and additionally to Figure 2, I have shown an initial station A which represents a sector or area at which process material is delivered. A clam shell bucket 9 handled by a crawler mounted mobile lift crane or an electric overhead traveling crane (handling device not shown) or a dump truck 10 may, as shown in Figure 2, be employed to deliver the process material or burden (a) upon a roller screen table or bed 12 (see also Figures 6 and 6A).

50 55 The screening cross-positioned table 12 is shown in an inclined position to receive the burden (a) from an upper, inclined chute portion 11 and to discharge oversize slag or debris of plus 12 inches mesh size, as shown, along a lower, front chute 13 upon a side-positioned, longitudinal, continuously-forwardly moving apron conveyor 15 that may be driven by a suitable motor (not shown). Material or burden of minus 12 inches in size drops downwardly through the grid openings or passes of the table 12, into a downwardly-converging chute 14.

60 65 Process burden or material of a larger size group, shown as plus 12 inches mesh size consisting of friable pieces of slag that has passed over the table of station A is, in effect, recycled back to the hopper 14 to join the undersize material along a longitudinal, continuously-moving, side-positioned, return-belt conveyor 28 and chute 28a, after (as shown in Figure 1a) it has been impacted or broken-up at a transverse station B by rotary impactor-crusher 40.

70 Referring particularly to Figure 3 of the drawings, the burden or process material from station A that has

passed through the roller screen apparatus 12 (shown as minus 12 inches mesh size) and the broken material returned from station B by conveyor 28 and chute 28a, moves down the inclined bottom chute 14 onto a vibrating feeder apparatus 26 that is shown energized by an electro-magnetic vibrating unit 26a. In this connection, see the commercial Jeffrey-Traylor feeders, as set forth in the 1951 catalog 830 of the Jeffrey Manufacturing Company of Columbus, Ohio. The apparatus 26 thus serves under the hopper as a forward feeder to discharge and distribute the process burden substantially evenly upon the main belt conveyor 27. The vibrating unit 26a is shown resiliently supported on a stand 26b and the front portion of the feeder apparatus suspended from an overhead support member 26c by a pair of adjustable resilient hangers 26d.

I have illustrated in Figures 4 and 4A, a typical impactor apparatus constructed in accordance with my invention. As shown in Figure 4, the larger size burden carried by the apron conveyor 15 is discharged therefrom into a forwardly-downwardly-inclined, upper feed chute 41 of the first rotary impactor-crusher 40 (see also Figure 1a) at station B.

In Figure 4, the chute 41 is shown bolted to a metal plate housing 42. The housing 42 has suitable handling tabs 42a and 42b (see also Figure 4A), and along the reaches of its front impact end wall is provided with a shock-absorbing liner or intermediate layer 43, such as of wood. The housing 42 is lined along its inner impact end wall by a series of abutting, side-stacked, steel billets 44 that are held in position by vertical end grooves provided along the opposite side liner plates 44a. The housing is lined along its opposite sides and top by heavy metal plates 44a, such as of abrasion-resistant steel, that are suitably secured in position to outer members of the housing, such as by stud bolts welded to the liner plates and projecting through suitably positioned holes in the housing.

The feed end of the apparatus 40 has a metal, outwardly-projecting, angle-shaped, back end box wall 45 that carries a removable end cover 46 that is held in position thereon by suitable threaded bolts 46a. A downwardly-inclined guide plate member 48 has an upper pair of projecting, back-mounting lugs or ears 48a that are secured pivotally to opposite sides of the box 45 by pivot pins 48b. Bars 47 fastened to opposite sides of the box are provided with a series of holes to alternately receive bolt and cotter pin assemblies that are termed adjustment side bolts 48d that are fastened through a pair of backwardly-mounted lugs 48c to opposite sides of the box. It will be noted that the pivot is at the upper end of the guide plate member 48 and that the adjustment bolts 48d are carried adjacent its lower end, so that the inclined positioning of the guide member 48 may be varied between the dot and dash positions (b) and (c) of Figure 4. The adjustable guide member 48 is shown provided with an abrasion resistant steel plate wear surface 49 bolted or otherwise secured onto its top face. The cover 46 may be removed, so that adjustment of the guide plate 48 may be easily accomplished by moving the adjustment side bolts 48d to suitable, oppositely-aligned notches or holes in the side bars 47.

When the guide member 48 is in its uppermost position (b), it delivers the burden more forwardly of the impact rotor or impeller means or wheel 50 (in the direction of its shown counterclockwise rotation). Conversely, when the guide member 48 is in its lowermost or greatest inclined position (c), it delivers the burden more towards the back of the rotary impactor 50. For larger and heavier materials, the adjustment is more toward the latter position and for smaller size materials, it is advanced or pivoted to an "up" or more forward position. In any position it provides at least a substantially tangential delivery of the materials to and from the peripheral surface of the impactor means 50.

Energy of impact is transmitted to the material by the rotary wheel or impactor means 50. As shown in Figure 4, the peripheral surface of the impactor 50 is protected by an abrasion-resistant steel facing 51 of suitable thickness. Radially-positioned mounting slots 50a project outwardly toward the cylindrical surface or face of the impact rotor 50 and correspond in number and spacing to the desired spacing and number of impactor blades or elements 52, which are constructed of an alloy steel such as a molybdenum-silicon alloy. For rotor balance, the blades 52 are equally spaced peripherally around the rotor and are shown secured in place by inset pins and wedges or key elements 53. The key elements 53 are carried beneath the facing 51 in stepped, slotted portions 50b, so as to protect them from the burden during the rotation of the wheel or rotor 50.

As shown particularly in Figure 4, the outer metal housing of the impactor 40 is bolted together. The top of the housing and lining 44a is readily removable by unbolting and lifting on the lugs 42a for maintenance access to the interior of the machine. The burden after impacting falls downwardly through a lower open end portion of the metal enclosure 42, onto a downwardly-converging discharge chute 54, and upon a suitable conveyor which, in the case of station B, is the return belt conveyor 28.

As shown particularly in Figure 4, the rotary impactor wheel or rotor 50 is secured on a drive shaft 55 by key means 56 to rotate therewith. The shaft 55 extends at its opposite ends through opposite, removable, end-slotted side plates of the housing 42, and is rotatably supported with respect thereto by side bearings 57. The opposite end portions 55a and 55b (Figure 4A) extend through bearings 57 which are mounted on spacer blocks 57a, and the end shaft 55a carries a V-belt drive wheel 58 that is keyed or secured to the shaft to thus drive the rotor 50. A motor-driven side-positioned belt (not shown) is adapted to engage the wheel 58 and drive it at a suitable speed. It may be noted that the impactor-crusher or rotor 50, its shaft 55a, and its bearings 57 may be removed as a unit by removing front end plate 42' (see Figure 4), removing bearing stand bolts 57b (see Figure 4A), spacer blocks 57a, dropping the unit down on side rails 57c, and rolling the rotor assembly out through the end of housing 42.

Figure 5 is a fragmental illustration of belt conveyor 29 at station D (see Figure 1b) feeding an impactor 40a of the same type illustrated in Figure 4, and is taken along the line V—V of Figure 1b. This type of belt conveyor feeding to the impactor 40a is also employed in connection with the impacting operations conducted at subsequent stations H and K of Figure 1b by impactors 40b and 40c respectively.

Screened burden or process material of a proper size 55 range, as shown in Figure 1a, of minus 12 inch size, which includes slag and metal, is shown continuously advancing forwardly from station A on belt conveyor 27 to station C of Figure 1b. Station C consists of a roller screen 12a of a type, such as shown in Figures 6 and 6A 60 of the drawings, having a suitable size of grid or pass opening. In Figure 1b, the passes of screen 12a at station C are shown as 6 inch mesh size.

At station C, the larger size portion of the burden (the oversize as indicated of 6 to minus 12 inches mesh 65 size) is discharged from a chute similar to chute 13 (see Figure 6) onto a continuously-moving conveyor 29 (see Figure 1b) for impacting at station D. The smaller size portion (the throughs as indicated of minus 6 inch mesh size) passes through the screen 12a and is discharged by 70 a chute similar to chute 14 (see Figure 6) onto the longitudinal, forwardly-moving belt conveyor 27a that carries it to roller screening station G. Material from the impactor 40a at station D, shown as consisting of 6 to minus 12 inch clean metal (which has been cleaned but 75 not broken) and minus 6 inch slag (which has been

broken by impacting) is returned along a transverse, continuously-moving, return belt conveyor 29a and fed onto the screen bed of a roller screen 12b at station E.

This screening at station E discharges, as oversize, clean metal (as indicated) of about 6 to minus 12 inches mesh size along a forward chute similar to chute 13 (see Figure 6), upon a transverse, continuously-forwardly moving belt conveyor 29b, and from it onto a longitudinal, continuously-moving, side-positioned, clean-metal-carrying belt conveyor 32. Thus, at this point of the process, the first separating-out of the clean metal content of the burden is effected by screen separating it as oversize from the remainder of the burden which includes smaller size slag and smaller size metal.

At station E, the smaller size portion of the burden (the throughs shown as of minus 6 inches mesh size) is discharged by a chute similar to chute 14 (see Figure 6) of its roller screen apparatus 12b upon the forwardly-moving conveyor belt 27a to combine with the throughs of the same maximum size from station C. The belt conveyor 27a advances the now-combined smaller size burden to another roller screen station G having a screen 12c of smaller screen size than the screens 12a and 12b at stations C and E respectively. At station G, the smaller size portion (the throughs indicated in Figure 1b as minus 3 inch slags and metals) is fed from station G onto a longitudinal, continuously forwardly-moving belt conveyor 27b which deposits the material onto a screen J' at station J. The larger size portion of the burden (shown the oversize as 3 inch to minus 6 inches mesh size) of screen 12c at station G is delivered onto a side-positioned, continuously-moving belt conveyor 30 which carries it to an impactor 40b at station H. The impacted burden from station H (shown as consisting of 3 inch to minus 6 inches mesh clean metal and minus 3 inch mesh size slag) is returned on the side-positioned transverse, continuously-moving, belt conveyor 30a to a 3" mesh roller screen 12d at station I.

At station I, the larger size portion of the burden (the oversize from screen 12d), which is shown as now consisting of 3 to minus 6 inches mesh clean metal, is discharged onto a transverse, continuously-forwardly-moving belt conveyor 30b, and then onto the longitudinal, clean-metal-carrying conveyor 32. As indicated, the roller screens 12c and 12d at stations G and I are the same size. Also, as shown, 3 inch to minus 6 inches mesh size clean metal is screen-separated from the other portion of the burden (shown as consisting of minus 3 inches mesh size slags and metals). The smaller size (the minus 3" mesh size "throughs" of screens 12c and 12d) burdens from stations G and I are combined on conveyor 27b and advanced forwardly to the vibrating screen J' at station J.

As shown particularly in Figures 6 and 6A, a roller screen apparatus is provided in accordance with the principles of my invention that, in effect, is a modified type of rotating grizzly that is side-balanced as to its driving means. The roller screen apparatus 12-12d as used at stations A, C, E, G, and I, comprises a suitable structural housing 20 that is provided with an upright support frame structure 24 and cross-connecting support members 23. The shafts of a series of cross-rollers 22, which define the inclined roll table, pass through dust seals 20a into bearings 21 within the housing structure 20. As shown, the rollers 22 provide a series of passes along the length of the bed through which the undersize portions of the material may pass. The shafts of two of the rollers 22 are driven through a pair of V-belt drive wheels or pulleys 15 and 15a, by a set of V-belts 16 from a motor-driven V-belt pulley or wheel 15b (see also Figure 6B). The drive wheels 15 and 15a are of larger diameter than the motor-driven wheel 15b to provide a speed reduction effect as to the actuation of the rollers.

It will be noted that alternate rollers 22 are driven

from one side of the apparatus by the wheel 15, through extended drive shaft 17, sprocket wheels 18, and sprocket chains 19. Other rolls 22 are driven by the wheel 15a and extended drive shaft 17a along the opposite side of the apparatus by sprocket wheels 18a and sprocket chains 19a (see particularly Figure 6A). Starting at the top or entering roll of the screen apparatus, each succeeding roll 22 is driven at a progressively faster speed than the preceding roll by the use of progressively smaller drive sprockets, so that the oversize material will feed smoothly across the roll table and will not clog or jam the grids or roll passes. As previously noted, the undersize portions of the burden pass through the roll pass openings or mesh of the roll table.

As shown on Figures 1b and 1c, I prefer to use electric vibrating screens J', L', O', P' and R' at stations J, L, O, P, and R respectively where the screen mesh size to be used is 1 inch or smaller. I have somewhat diagrammatically illustrated an electric vibrating screen P' in the left portion of Figure 10 of the drawings which is employed at station P. In Figure 9 of the drawings, I have shown screen O' which is employed at station O. Each of the screens O' and P' is  $\frac{3}{8}$ " mesh.

The vibrating screen apparatus as shown in Figure 25 10 has a supporting frame structure 60, resilient support rod assembly or structure 61, a downwardly-declining upper feed or input plate 62, a downwardly-declining vibrating screen table or screen feed trough member 63, on which is mounted a wire screen 63a of suitable mesh size, an under-delivery outlet chute 64 for smaller size material, an end-delivery, outwardly-declining, bottom guide or outlet plate 65 for larger size material, and an electrically-activated magnetic vibrator unit 66. Screens of this type are available commercially, such a unit being manufactured by the Jeffrey Manufacturing Company of Columbus, Ohio. The table 63 is pivotally suspended near its upper end by the adjustable side rod structure 61. The rod 61a passes through a cross frame member 61b. A resilient member 61c is interposed between the cross frame member and a nut 61d secured to the rod. The vibrator unit 66 is secured to the sides of the screen table adjacent its lower end and is pivotally suspended from the frame structure 60 by a pair of pivotally-mounted, side-positioned hangers 61c. Each hanger 61c is provided with a turn-buckle to adjust its length.

Referring again to Figure 1b, the smaller size burden of minus 3 inch slag and metal which is carried forwardly by belt conveyor 27b, is delivered to the vibrating screen J' at station J at which the smaller size portion of the burden (as indicated, of minus 1 inch mesh size) passes through the screen and onto the longitudinal, forwardly-advancing, continuous belt conveyor 27c. The larger size portion of the burden (the "overs," as indicated, of 1 inch to minus 3 inch material) containing both slag and metal passes across the vibrating screen J' of station J and discharges onto a transverse, side-positioned, continuous belt conveyor 31. The conveyor 31 delivers its burden to a rotary impactor crusher unit 40c at station K from which it is returned on a transverse, side-positioned, continuous belt conveyor 31a to a vibrating screen L' at station L. At station L, the clean metals, as represented by the larger size portion of the burden (shown as of 1 inch to minus 3 inch mesh size) pass across the screen onto a transverse, continuously-forwardly moving, belt conveyor 31b, and then to the main longitudinal, clean metal-carrying, belt conveyor 32. The smaller size portion of the burden at station L (the "throughs" from screen L' shown as minus 1 inch mesh size) is discharged upon the forward conveyor 27c and thus, combines with the same smaller size burden from station J.

Referring particularly to Figures 1b and 7, clean metal of a size range of 1 to minus 12 inches mesh size that has been delivered from stations E, I, and L, is combined on the clean metal-carrying conveyor 32 and carried by

such conveyor to a magnetic head pulley station F. At this station, magnetic pulley 70 (see Figure 7) delivers magnetic portions of the metal burden backwardly along one side of an inverted V-shaped chute wall 71 onto a transverse, side-positioned, continuously-moving belt conveyor 32b. The conveyor 32b is shown as delivering the magnetic, clean metal of the indicated size range to a suitable collecting area (3), see Figure 1b. The non-magnetic portion of the clean metal is delivered forwardly along the other side of the chute wall 71 onto a longitudinal, continuously-moving, belt conveyor 32a which carries it to a transverse, side-positioned, continuously-moving belt conveyor 32c. The conveyor 32c is shown as delivering the non-magnetic portion of the clean metal to a suitable collecting area (2) see Figure 1b.

As shown in Figures 1b and 1c, the combined smaller size portions of the burden from stations J and L is carried forwardly by the conveyor 27c to a magnet station M. This station is somewhat diagrammatically shown in Figure 8 of the drawings. A self-cleaning, rectangular, electro-magnet 73 of a type commercially available has a non-magnetic guard 74 on its bottom face over which a cleated rubber belt 75 continuously moves transversely of the direction of movement of burden along the conveyor 27c. The belt 75 is carried by an adjustable belt idler pulley 76 and a belt drive pulley 77. The drive pulley wheel 77 has a sprocket that is actuated by drive chain 78 and gear motor 79. The magnet 73 and the balance of the assembly are suspended from a supporting member 82 which carries suspended support hangers 81. At station M, the magnetic portions of the burden that are being advanced forwardly by the belt 27c, are attracted by the magnet 73 and are carried by the cross belt 75 to a side delivery chute 83 (see also Figure 9). As shown in Figure 1c, this material is then delivered to a transverse, continuously-moving belt side conveyor 34.

The conveyor 27c, at its forward end, is driven through a magnetic pulley 85, see Figure 9 of the drawings. The pulleys 85 (and 70 of conveyor 32, see Figure 16 and Figure 7) may be high intensity electro-magnetic pulleys of conventional design and operation that are available commercially. At station N, the pulley 85 in cooperation with the conveyor belt 27c, which is of a suitable material such as rubber, effects a separation of the remaining magnetic material from the balance of the burden and delivers the magnetics thus removed to a main down-chute portion 83a of the chute 83, combining with the magnetics removed at previous station M and being deposited on the transverse, side-positioned, continuous belt conveyor 34.

That portion of the burden with insufficient magnetic attraction to be removed at stations M or N is discharged forwardly onto the upper guide member 62 (see Figure 9) of a  $\frac{3}{8}$ " mesh vibrating screen apparatus O' previously described in connection with Figure 10. When it is desired to further process the burden being fed by guide member 62, swing guide member 67 is positioned in the inclined, full-line position of Figure 9, in alignment with the guide member 62, to feed the burden downwardly through an opening defined by a feed chute wall 62a upon the bed 63a of the vibrating screen apparatus. The swing guide member 67 is pivotally mounted at 67a to sides of the chute 64, so that it may be swung to close off the passageway or opening with respect to the guide wall 62a (dot and dash line position of Figure 9), and to discharge the material directly into the down chute 64, through a bottom opening that is provided. However, as previously pointed out, when the member 67 is in its full line position of Figure 9, all the material is delivered to the vibrating screen bed 63a. The material of a size (shown as of minus  $\frac{3}{8}$  of an inch mesh in Figure 1c) small enough to pass through the screen O' falls downwardly into the chute 64 and is discharged therefrom upon a transverse, side-positioned, continuous, belt conveyor 33b that is employed to carry

non-magnetic slags and magnetic slag rejects to a suitable disposal or collection area (4), see Figure 1c.

The material of larger size (minus 1 inch to  $\frac{3}{8}$  inch mesh) which passes across screen O' as oversize (see Figure 9) moves down bottom guide 65 into the pass (shown in Figure 1c as  $\frac{3}{8}$  of an inch) of a roll crushing apparatus 160 having a pair of rotating crusher wheels or rolls 88. It will be noted that the rolls 88 define a down-pass and are rotatably carried in a housing 87 for continuous rotation by a suitable motor and drive (not shown). The material that is crushed in the pass defined between rolls 88 is then delivered from a down-chute 89 to a transverse, side-positioned, continuous, belt conveyor 35.

Referring again to Figure 1c, the material from the roll crusher 160 delivered to conveyor 35 (as indicated of minus  $\frac{3}{8}$  inch mesh size) is transferred through a suitable chute to a longitudinal, continuously-moving, backwardly directed conveyor 35a and hence to a transverse, side-positioned, continuously-moving, belt conveyor 35b, and from conveyor 35b back to the main longitudinal conveyor 27c.

Magnetic material which is delivered to the side belt conveyor 34 (see Figure 9) is carried to vibrating screen P' at station P and is there separated into two size groups or portions, the smaller size portion (shown as minus  $\frac{3}{8}$  of an inch mesh) is delivered to a longitudinal, forwardly-moving, continuous, belt conveyor 27d, see also Figure 10. Referring particularly to the latter figure, the larger size material (the "overs") is delivered from station P to station Q along front guide plate or member 65 onto a transverse, continuously-moving conveyor belt 34a.

At station Q, see particularly Figure 10, the burden or material is carried by the conveyor belt 34a beneath a series of alternate north and south magnet poles of a magnet unit 90 and a continuously-moving, non-magnetic belt 91 of a suitable material, such as rubber, which is moving in the same direction as conveyor belt 34a. Apparatus comprising the unit 90, conveyor 34a, and the belt 91 may be obtained commercially and is termed a Ball-Norton, self-cleaning type of magnetic separator, such as supplied by Ding's Magnetic Company of Milwaukee, Wisconsin. By adjusting the D.C. current input from a D.C. current source (not shown) to the magnet unit 90 by means of a rheostat or variable resistance (not shown) wired in series with unit 90 and by adjusting the spacing between belt 91 (including magnet 90) and conveyor 34a (means of adjustment not shown), magnetic material of insufficient cleanliness or purity is either not lifted from belt 34a or falls from belt 91 before reaching the apex of chute 93. Material of lesser magnetic attraction is thus carried by the belt 34a forwardly or falls from belt 91 before the end travel is reached to discharge upon the left half of the downwardly-declining V-shaped diverter chute or guide member 93. Material having suitable cleanliness and purity and thus high enough magnetic attraction is propelled forward by belt 91 and discharged onto the right half of the diverter member or chute 93 and then onto a longitudinal, continuously-forwardly-moving belt conveyor 36.

The lesser magnetic portion of the material (of size range minus 1 inch to  $\frac{3}{8}$  of an inch) is delivered to the pass (shown in Figure 1c as  $\frac{3}{8}$  of an inch) of the rolls 88 of a roll crusher and is discharged by down-chute 89 upon a longitudinal, continuously-moving, backwardly-directed conveyor belt 35c which carries the material to transverse conveyor belt 35b (see Figure 1c) to combine with the discharge from conveyor belt 35a. Both are then returned to forwardly-moving, longitudinal belt 27c, so that the magnetics cleaned and/or released by the crushing operations may be recovered by recycling.

As shown in Figure 1c, clean metal particles and high iron content slags and metal oxides which are delivered to the forwardly-moving belt conveyor 36 from the magnetic separator 90 (see Figure 10) are, in turn, delivered to a transverse, side-positioned, continuously-moving

belt conveyor 36a, and then to a suitable delivery or collecting area (5).

The smaller size magnetic material (the "throughs" from screen P' shown as minus  $\frac{3}{8}$  of an inch mesh) being carried forwardly by conveyor 27d is delivered to vibrating screen R' at station R that is similar to the screen P' at station P, but is shown as having a smaller size mesh of  $\frac{1}{8}$  of an inch. The larger size portion of the burden separated at screen station R (shown as minus  $\frac{3}{8}$  to  $\frac{1}{8}$  of an inch mesh size) passes across the vibrating screen R' of station R as oversize (see Figure 1c) to a station S that is similar to that described in connection with station Q of Figure 10. The magnetic apparatus of station S delivers the lesser magnetic material to a roll crusher which has a pass of  $\frac{1}{8}$  of an inch, so that delivery to return conveyor 35c is material of minus  $\frac{1}{8}$  of an inch mesh. The more magnetic material from station S of controlled purity and cleanliness (shown as minus  $\frac{3}{8}$  to  $\frac{1}{8}$  of an inch) is delivered to the forwardly-moving belt 36 to combine with the product from station Q. As indicated on Figure 1c, the material thus delivered to the storage area (5) is of a  $\frac{1}{8}$  to minus 1 inch mesh size of clean metal and high iron content magnetic slag and oxides which is of a type and size suitable for direct blast furnace utilization.

The smaller sized material screened out at station R (shown as minus  $\frac{1}{8}$  of an inch mesh) which passes through the mesh of the vibrating screen, is delivered to a longitudinal, continuously forwardly-moving conveyor belt 27e, and from it to magnetic separator station T. Reference is made to Figure 11 which shows the operation of station T. It will be noted that the magnetic separating unit is of the same type of unit previously described in connection with Figure 10. Details of the drive of its feed belt 27f and its cooperating separator belt 91 are shown. That is, gear motor 95 actuates a drive chain 96 which cooperates with a sprocket on one of the pulleys of belt 91, an idler sprocket 92, and a sprocket on one of the pulleys of belt 27f to simultaneously actuate them.

The lesser magnetic portion of the burden which is delivered by the conveyor 27e to the magnetic separating unit of station T falls downwardly through a chute 94a upon a transverse, side-positioned, continuously-moving belt conveyor 33, while the higher purity magnetic material is discharged downwardly through a chute 94b onto a transverse, side-positioned, continuously-moving belt conveyor 37. At this point, see Figure 1c, the high purity magnetic metal particles, slag, and metal oxides are shown as minus  $\frac{1}{8}$  of an inch in mesh size, and the side belt conveyor 37 carries them to a delivery or collecting area (6) from which collecting point they may be delivered to a sintering plant for agglomeration to prepare them for suitable use such as in a blast furnace. The impure magnetic rejects, less than  $\frac{1}{8}$  of an inch mesh size, are carried by conveyor 33, to conveyors 33a and 33b, and thence to the disposal area (4).

#### Further considerations

It should be noted that my system or procedure has been developed, not only from intensive study, analysis and research into the physical properties and chemical analyses of the materials to be processed involving critical and important factors which I have determined must be recognized and properly controlled, but also from the standpoint of a careful study of steel plant operating practices and experimental work which has involved the design, testing, arrangement, and utilization of various types of processing apparatus or equipment for each successive and progressively coordinated parts of the operation and for the particular nature and size of the process burden or material mixture involved at the various stages of the processing sequence.

As determined in these studies, there are many factors

that enter into the problem that had to be considered and met which importantly include the very wide size range of the starting process mixture, its highly abrasive nature, its highly mixed characteristics from the standpoint of 5 crushability of the portions thereof that are to be separated, the similar and dissimilar magnetic characteristics of the various portions, as well as the agglomerated or bound nature of a large proportion of the metal and metal oxide content of the burden which is to be processed.

10 Less obvious, but highly important are the various detailed facts which I have discovered in my studies relative to each of the components of the mixture.

For instance, I have determined that the metal content 15 of individual pieces of open hearth flush or runoff slag varies from a minimum of 2 to 3 percent to a maximum of 15 to 20 percent, and that there is generally insufficient magnetic metal present in flush slag, even at the higher metal contents to render the metal pieces capable 20 of being picked up or removed from a process mixture by commercially practical high intensity magnetic equipment. Furthermore, I have determined that a large amount of the embedded metal content of flush slag is under 1 inch in size and is concentrated to a large extent 25 in a size range from  $\frac{1}{20}$  of an inch to  $\frac{3}{8}$  of an inch. Although a great number of metal particles are present below  $\frac{1}{20}$  of an inch in size, the quantity present has been found to be normally not great enough in total weight to justify specific procedures for their recovery as such.

30 However, I have discovered that if a high percentage 35 of total metal content is to be recovered, it is necessary to break down these pieces of flush slag and to increase the metal-slag matrix ratio of the smaller pieces. I have discovered that high velocity impact breaking is effective 35 for reasons which will be later discussed in shattering the bond and effecting cleavage between the metal particles and the slag matrix to accomplish the desired results. In addition, I have determined that it is necessary to 40 reduce and limit the maximum piece size of material in the burden before high intensity magnetic means can be used to effectively and completely recover the magnetic metal content on a continuous basis.

In this connection, it should be noted that the effective 45 field strength and pick up ability of any given magnetic device is directly related to the distance between the magnet face and the center of gravity of the magnetic piece or object to be picked up. Further, if magnetic material is to be continuously picked up or removed by a magnetic device from a continuously-moving burden 50 containing mixed sizes, such as from a burden on a moving rubber conveyor belt, the face of the magnetic device suspended above the burden would have to be located a distance from the conveyor belt equal to at least twice the largest piece size in the burden, assuming the burden 55 depth does not exceed the size of the largest piece. This is necessary in order to avoid interference or jamming between the magnetic material which is attracted to the magnet face and the burden flowing or passing under it.

Thus with a maximum piece size of 1 inch in the burden, 60 it would be theoretically possible, if the burden depth was not over 1 inch, to operate an overhead magnetic device with the magnet face a minimum of 2 inches from the conveyor belt. This would mean that the center of gravity of a small magnetic particle on the 65 surface of the conveyor belt would be a maximum of 2 inches from the magnet. By similar reasoning, it can be understood that with a 6 inch maximum piece size, the face of the magnet would have to be at least 12 inches from the conveyor belt and from the center of 70 gravity of a small particle on the belt. With 12 inch maximum piece size material, this distance would necessarily increase to 24 inches for a continuous overhead removal system. Thus, if proper separation or removal of magnetic material from a mixed burden is to be 75 effected, it is obvious that maximum piece size of the

burden is an important and critical factor and should be reduced to the greatest practical extent.

Although attempts have been made to apply magnetic fields and remove magnetic material from the underside of a continuously moving burden, such as through the use of magnetic head pulleys on a belt conveyor, in an effort to combat or overcome this distance problem, the results are not satisfactory in mixed burdens of the type under consideration. Due to the difficulty of retaining irregular shaped pieces of relatively low average magnetic character on a magnetic pulley face with a simultaneous heavy flow of non-magnetic material passing over the pulley, there is a definite loss of recoverable metal and magnetic materials, particularly in the larger sizes, which increases as the maximum piece size of the burden increases.

In addition to the necessity of reducing burden piece size and increasing the metal-slag matrix ratio, as mentioned above, to enable substantially complete magnetic separation of the metal and magnetic material content of the burden, it is also important to clean the metal and remove in a substantially complete manner the flush slag that will adhere to or be imbedded in the irregular crevices or pockets of the metal pieces. This is important, when the metal is of a larger size (over 1 inch) to be re-used in an open hearth furnace, in order not to return useless slag to the furnace to be re-melted, but it is of even greater importance in the smaller size metal (under 1 inch) which is to be re-used in a blast furnace, in order to maintain low phosphorous content in the recovered product. The necessity of properly cleaning the small metal particles becomes more apparent when it is realized that open hearth flush slag contains 1 to 2 percent phosphorous content, whereas desirable charge metallics to a blast furnace should contain not more than 0.2% phosphorous, in order that the iron which will be produced from the furnace does not have excessive phosphorus content.

In this connection, I have discovered that if the large metal pieces, down to say 1 inch, are properly impacted at a high enough velocity, a cold working of the metal occurs which effectively breaks the bond between the metal and the adhering and embedded slag material, thus cleaning the metal without abrasion loss of metal or reduction in metal piece size. In the smaller size ranges, below 1 inch, essentially the same result is accomplished by cold rolling the metal particles  $\frac{1}{8}$  of an inch and larger through the pass rolls of a roll crusher. Again it should be noted that, although the smaller particles may be distorted in shape by this procedure, there is no reduction in size or loss of metal due to abrasion.

In contrast to these procedures, other methods which might be attempted for cleaning this metal, such as barrel tumbling, are not suitable or effective, would be prohibitively expensive to operate and maintain, and, if carried to an extreme and thoroughly uneconomic point at which substantially clean metal might be produced, would result in a considerable size reduction of the metal pieces and an excessive overall loss of metal due to abrasion.

Another component of the process mixture, whose detailed physical properties and chemical composition should be considered, is open hearth tap or finishing slag.

I have discovered that tap slag, although it appears to be a tough, uniform or homogeneous material, actually is a very friable material and is made up of small individual particles which vary widely in magnetic characteristics and chemical analysis.

Originally I discovered a variation in magnetic characteristics within a small specially prepared 1 inch cube of this material. Later, after discovering the very friable nature of this material, I was able to crush individual pieces of tap slag and by magnetic means separate the crushed material into various magnetic fractions or component portions. I then discovered through chemi-

cal analysis of the component portions that various fractions of the crushed material from a single piece of slag, varied in iron content from as low as 2.5% Fe to as high as 52.1% Fe. I also discovered that the phosphorous content of this material varied from 0.48% to 0.23%, and that the highest phosphorous content and lesser magnetic properties were associated with lower iron content. Thus, I discovered that by crushing open hearth tap slag, not only would it be possible to separate it from magnetic metal by screening methods, but that crushing of this material would prepare a substantial portion of it for recovery and concentration by magnetic means for ultimate use as a blast furnace charge material. It was also determined that if this material was to be of maximum value, it should not be over-crushed. That is to say, the size of the tap slag particles should be reduced only to the extent necessary for their separation and magnetic concentration, in order that a majority of this material would remain above a minimum size ( $\frac{1}{8}$  of an inch) that is acceptable for direct re-use in a blast furnace.

Thus, by coordinating and correlating the information which I have discovered and evaluated relative to the effect of high velocity impacting in the cold working of metal and its resultant effect in shattering the slag-metal bond, and the physical and chemical properties of open hearth slags which I also have discovered, I developed my unique and novel procedure of impacting and screening mixtures of these materials to effectively clean and separate the larger metal and simultaneously prepare the embedded smaller metal and magnetics for a fully effective and substantially complete recovery at a later stage of the process. Not only did this technique enable a desired complete separation of magnetic metal and magnetic slags which had heretofore been impossible, even by hand sorting, but it also provided a means for recovery and cleaning of non-magnetic metals, with additional important benefits accruing from this technique to the balance of the process burden.

It should be noted that the breaking-up stages or steps in the complete process, as illustrated, including attendant selective scrap or metal recovery, preferably involves by-passing of fine material, progressively increasing the severity or speed of impact, as the size range of the material decreases, and that magnetic separation is deferred until the size range or maximum piece size of the burden has been reduced sufficiently to enable effective magnetic separation, and until essentially all of the non-magnetic scrap has been removed.

In carrying out my invention, to release and recover clean metal of an open hearth and electric furnace charging type, I found it necessary to develop a rotary impactor apparatus having special characteristics which are different from those of commercially available apparatus. For example, I avoid, as much as possible, shear of the material by the rotor blade as distinguished from break-up of the material by impacting, and I impart as high a kinetic energy as possible to the incoming material and increase its velocity of impact against a specially reinforced breaker wall. Thus, I enter the material or burden of a selected size range on the impeller or impactor rotor, near its top or upper sector or half, rather than the lower sector or half. This not only imparts maximum kinetic energy or momentum to the pieces or particles to continue essentially in their original direction of movement and impinge with maximum velocity upon the well reinforced, shock-resistant liner of the impactor (as contrasted with upwardly upon the roof or top of the housing), but also minimizes wear on the rotor surface and blades to the extent that the use of this part of the apparatus becomes practical. Billets of carbon steel backed with an oak wood liner have been found to provide a good impact wall lining which transmits a minimum of impact stress to the external shell of the machine.

The blades of the impeller rotor should be equally

spaced for rotor balance, and for slower speed operation on larger material will be preferably three or four in number. They are keyed into position on the rotor for ease of replacement. As mentioned previously, these blades are not employed as shear elements, but as movement-accelerating and momentum-imparting means for the pieces of burden or process material. It is highly important in this connection to minimize wear and tear on the apparatus, since the process is a continuous one and involves large malleable or relatively unbreakable materials, such as free metal, as well as the more friable materials, such as slag. If the impellor blades or impactor rotor have too fast a speed, open hearth tap slags will be over-crushed and the machine may also tend to be self destructive, both from the standpoint of impact shock and unnecessary wear; while too slow a speed may not properly clean the metal or reduce the friable portions of the burden down to the requisite size range for screen separation.

The angle of feed between the guide means and the rotor is also important for various size ranges of material, in order to enable acceleration of the material or burden to the speed of the rotor. For a given rotor, the smaller size material will have relatively instantaneous acceleration, since kinetic energy will be rapidly absorbed to increase its velocity, while the absorption of sufficient energy and velocity by the larger sized pieces of material will be somewhat slower. Thus, the guide means should be adjustable to provide a more forward point of entrance onto the rotor for smaller sized process material, while for larger material the guide means may be set at a steeper angle to provide a less forward position of entrance onto the rotor. As shown in Figure 4, I have provided a guide member 48 that is capable of adjustment in an angular relation to the horizontal; it may be varied by steps between about 35° to 55° for best results.

The free discharge opening of the impactor, including that portion defined by the impact end wall, the opposed side walls, and the peripheral face as generated by the rotating impeller blades, for exit of the material from the impactor apparatus, must be of sufficient size to readily or freely pass the largest piece of non-breakable material or malleable metal content of the burden without damage to the apparatus. For example, an opening of about 30 inches in dimension has been found operationally practical for passing metal up to a maximum dimension of about 24 inches in size (mesh passing); it may be noted that a 40 x 36 inches rotary impactor crusher complies with these conditions. As to a 40 x 36 inches crusher, I have reference to one having a rotor length of 36 inches and a rotor diameter across blade tips (diameter of maximum outer periphery of blade movement) of 40 inches. Further by way of example, a 24 x 24 inches rotary impactor crusher having about 10 inches clearance can be used for material of up to about six inches in size with an optimum of about three to four inches; and a 30 x 30 inches rotary impactor having a clearance of about 20 inches has been found to be practical for material up to about 12 inches in size. The clearances to which reference is made are those defined between the tips of the rotating impeller blades and the end impact wall within the housing. This is also true for the input feed opening. In this connection, it should be noted that I have importantly been able to employ a relatively large and unrestricted exit or discharge opening, and by controlling the size range of input material in relation to rotor speed, to completely break-up the friable material to a maximum size which is below a selected size range for separation of the larger pieces of metal. The metal content in the size range to be removed at the next screening station, is simultaneously freed or cleaned of slag, etc., by the high velocity impacting operation. This is highly desirable in order that the selected size range which is to be separated-out is of sufficient

cleanliness for direct charging into an open hearth or electric furnace.

As to Figure 1b, it should be noted that I have been the first, as far as known, to provide a recovery of both magnetic and non-magnetic clean metal from slag, and then to provide a separation of non-magnetic metal (e.g. stainless steel) from magnetic metal (e.g. ordinary carbon steel), as by magnetic pulley means, without the necessity of hand picking and cleaning, see collecting areas 10 (2) and (3).

It will be noted that impact crushing of burden and cleaning of metal is not shown for material under 1 inch mesh size. Although, rotary impactors can be used for material in this size range, the very high rotor speeds 15 which are required to obtain best results cause considerable rotor and blade wear. There is also an excessive crushing effect on the open hearth tap slags in this size range which I desire to avoid.

As indicated in Figure 1c, roll type crushing is preferred in size ranges below 1 inch and has been effectively used in the manner shown.

It should also be noted that the type of screening-out apparatus and procedure employed along the line or system is varied to accomplish a maximum effectiveness 25 and completeness of separation, based on the size of the burden at each station or step. For example, I employ a roller screen apparatus, such as illustrated in Figures 6 and 6A, for separating out larger size material 30 ranges until the mesh size to be separated reaches a size range that from a practical standpoint, may be accomplished through use of electric vibrating screens (for example 1 inch and smaller).

The roller screen apparatus of Figures 6, 6A and 6B has been found to be practical for screen separating 35 heavy burdens of process material from a minimum of about 1½ inches mesh up to 18 inches or more mesh size (12 inches maximum size shown in Figure 1a), and the magnetically vibrated screen apparatus has been found to be most successful where the screen mesh is 1 inch and 40 smaller. An electric vibrating screen is ineffective for large sizes because of the relatively short distance or stroke of vibration.

The slope of the bed of the roller screen apparatus to the horizontal may lie within a range of about 30° to 45 40°, and as an optimum, from about 30° to 35°. Such slope is necessary for efficient operation and to prevent clogging or jamming. The angle of inclination is also important from the standpoint of conveying material across the screen bed.

50 For the class of material being processed, the burden depth should not exceed two to three times the pass opening or mesh of the screen, but this will vary somewhat. For example, for a mesh or pass size of about 3 inches, a depth of burden of about 6 to 8 inches can be effectively processed. However, for a roller screen with a 12 inch pass size, burden depth should be limited to about 55 18 inches.

By employing a balanced drive on the roller screen with approximately half of the rolls driven from each 60 side and with speeds of the roll shafts increasing along the length of the screen toward its delivery end (progressively faster speeds forwardly along the table), and with succeeding rolls rotating in the same direction (opposite surface directions in the pass itself), I achieve 65 screening of large size material with a simple rugged device which requires a minimum of maintenance, does not necessitate heavy foundations, and has a relatively low power consumption. For instance, I use about a 3 horsepower motor to drive the roll shafts of a roller screen apparatus having a mesh or pass size of about 3 inches. Compared to this, an eccentric-actuated motor-driven, mechanical vibrating screen for the same pass opening would require a heavy foundation and supports, and a much larger motor and drive.

70 75 It will be noted that I prefer high intensity magnetic

fields applied from two separate directions to separate the magnetic portion of the burden from the non-magnetic portion. Referring to Figure 9, the magnet 75 applies a magnetic field from above the burden and the magnetic pulley 85 applies a magnetic field from below the burden. By high intensity magnetic fields, I mean the highest possible magnetic fields that it is possible to achieve using commercially practical magnetic equipment, such as is illustrated, operating at maximum allowable D.C. current flow in the case of electro-magnets. If permanent type magnets are used, I mean the highest intensity field strength permanent magnets which can be practically applied to this use. As previously noted, burden depth and maximum piece size in the burden are reduced to permit most effective use of the high intensity magnetic fields thus provided. By these means a maximum recovery of crude magnetic material can be effected. The use of two separate magnetic devices with fields applied to the burden from above the burden and below the burden is a preferred method of magnetic separation to assure maximum recovery, but the use of both is not essential, if some sacrifice in recovery can be tolerated or if the rate of material flow is substantially reduced.

The size separation of crude magnetic material and the unique use of controlled current magnetic separators in conjunction with roll crushing apparatus in a closed recycling circuit has been described. This novel arrangement permits rheostat control of product quality such as has never before been achieved, and in view of previously discussed facts with regard to the material being processed, should enable an understanding of the principles involved necessary to a complete control of iron content and phosphorous contamination in the refining and concentrating of the metallics for blast furnace use.

It should be noted that while a commercial Ball-Norton type of magnetic separator has been illustrated to separate high purity product from less pure magnetics, and that it is highly efficient and preferred for this purpose, by reason of the fact that its north and south poles are alternated along the length of the upper conveyor belt, it is nevertheless possible to obtain similar although not equal separating action by means of an ordinary self-cleaning rectangular magnet suspended over a conveyor belt operating "in-line" with the feed conveyor. Rheostat control of current to such a magnet together with control of belt spacing would be required similar to the Ball-Norton separator.

Again it should be noted that it would be possible to substitute other types of crushing devices in the refining stages of the processing to replace the designated use of roll crushers and accomplish a similar result. The use of roll crushing devices is however preferred.

With regard to the use of roll crushers or other types of crushing means other than of the rotary impacting type for reducing the size of non-magnetic slags and other materials containing larger sized pieces of non-crushable metal, it should be noted that types of crushing apparatus other than the rotary impactor type may only be employed in the manner illustrated after magnetic removal of the large metal has been effected.

#### Other exemplary procedures or utilizations

##### A

In some instances, steel plants may desire to use a limited amount of sized slag from their open hearth furnaces as a substitute for a portion of the limestone which is used as a flux in their blast furnace operations. The layout of Figure 12 illustrates an application of my invention to comply with such a requirement. In this illustration, non-magnetic slag is produced in a size range of from  $\frac{3}{8}$  to minus 3 inches, employing a cooperative arrangement and material flow as to final magnetic separating and refining, as illustrated. Thus, a complete arrangement of facilities may employ Figure 1a in full and

Figure 1b to the line Z—Z, so as to take the clean metal from the longitudinal conveyor 32 and deliver sized burden to conveyor 27'b for use in the system of Figure 12.

In Figure 12, magnetic separation is shown as effected when the burden is below 3 inches in piece size. Rotary impacting and screen separation is used to clean and separate about 1 to minus 3 inches magnetic metal from magnetic slag in the same size range. Subsequent refining stations for magnetics below 1 inch in size are shown as similar to the procedure of Figure 1c. Since slag over  $\frac{3}{8}$  of an inch is intended for re-use in the layout of Figure 12, a roll crusher is not required (as in Figure 1c) for further size reduction of the non-magnetic portion of the burden.

To facilitate an understanding of the layout of Figure 12, I have employed the same reference numerals for continuously moving conveyors and discharge areas as in Figure 1c, where the nature of the burden, direction of movement, and processing are the same as in Figure 1c; where they have a similar functioning, but employ a slightly different size or nature of material or operative relationship, I employ the same reference numerals with prime suffixes. The same is true as to the alphabetic references of the processing stations. Where the arrangement or utilization is different, I have employed new numerals and station letters.

A study of Figure 12 discloses that burden being advanced continuously-forwardly on conveyor 27b of Figure 1b, is moved by now-designated continuous belt conveyor 27'b to a self-cleaning, rectangular magnet station M' (see 75 of Figure 9) and to a magnet pulley station N' (see pulley 85 of Figure 9) at which minus 3 inches size magnetic slags and metals are discharged to a continuously-moving transverse or side conveyor 97. Non-magnetic slag is shown carried forwardly by conveyor 27'b to a vibrating screen station W (see vibrating screen equipment of Figure 9). At station W, non-magnetic slags of  $\frac{3}{8}$  to minus 3 inches are shown delivered over the screen table ( $\frac{3}{8}$  of an inch mesh) to continuously-moving side conveyor 33'b, and thence, to discharge or collecting area (4'), for example, for charging into a blast furnace.

On the other hand, as shown, the minus  $\frac{3}{8}$  inch non-magnetic slag portion of the burden passes through the screen of station W and is delivered to continuous, side belt conveyor 160. Conveyor 160 discharges on longitudinally-forwardly-moving conveyor 100a to deliver the material to a collection or discharge area (7). Minus  $\frac{1}{8}$  inch magnetic slag rejects are shown carried by continuously-moving side belt conveyor 33 from station T to conveyor 100a to thus combine with the minus  $\frac{3}{8}$  inch non-magnetic slag burden for delivery to area (7).

The minus 3 inches magnetic slag and metal burden that is segregated at station M' and N' is shown, on delivery to side conveyor 97, as carried to the screen table (see 63 of Figure 10) of a vibrating screen station U. At station U, 1 inch to minus 3 inch magnetic slags and metals are shown as passing over the screen (1 inch size mesh) and as advanced by longitudinal, continuously-moving belt conveyor 98 to a rotary impacting or breaking-up station V (see the apparatus of Figure 4). The resultant broken-up burden is then shown delivered from station V to a continuously-moving side belt conveyor 99, and at this time, consists of minus 1 inch magnetic slags and minus 3 inches magnetic metal. The burden from conveyor 99 is shown delivered upon the screen table (of 1 inch mesh, see 63 of Figure 10) of vibrating screen station L'. As illustrated, 1 inch to minus 3 inches clean metal is carried over the screen of station L' and delivered to continuously-moving side conveyor 31b to combine with the burden of clean metal return conveyor 32 (see Figure 1b) and metallics under 1 inch in size pass through the screen of station L' and are returned to conveyor 27'b for recycling. It will be

noted that the burden of 31b is of the same type and size range as conveyor 31b of Figure 1b.

As shown, the burden of conveyor 34 from station U of Figure 12 is of the same size and content as the burden of conveyor 34 of Figure 1c and is processed in the same manner with reference to stations P, Q, R, S and T of Figure 12 as at the same stations of the layout of Figure 1c. It will also be noted that the burden delivered at areas (5) and (6) of Figure 12 is of the same size and nature of content as corresponding areas of Figure 1c. Briefly, the difference between the final process system of Figure 12 and Figure 1c rests in the fact that the initial burden of Figure 12 is of a larger size content, and is first, magnetically separated-out to provide a relatively larger size of non-magnetic slags at delivery area (4'). In Figure 12, the remaining magnetic content or portion is then subjected to rotary impacting to make possible the removal of 1 to minus 3 inches size of clean metal. Also, in Figure 12, the smaller size slags are delivered to a separate delivery area (7).

## B

Some steel plants do not have electric furnaces and thus, do not produce non-magnetic steels, such as stainless steel. In addition, a larger size range of non-magnetic slag may be desired for blast furnace use, along with different size ranges of clean metal and refined metallics for open hearth and blast furnace use. To illustrate such an application, reference is made to the layout and procedure of Figure 13.

In an operating situation such as is illustrated in Figure 13, it is assumed that the amount of plus 12 inches material to be broken is either negligible or present in such a limited amount that a ball-dropping operation may be economically employed in place of the pre-processing facilities of Figure 1a. Since non-magnetic slag is to be sized and produced in a 3 to 6 inches size range, and since no non-magnetic metal is present, only one impacting and screening or segregating operation is shown utilized prior to magnetic separation. It should also be noted that in the single impacting step which is shown employed on a 3 to 12 inches size burden, the more friable magnetic slags are shown reduced to about a minus 3 inches size, while the lesser friable non-magnetic slags are shown reduced to about a minus 6 inches size range. Thus, screen removal of clean metal after such an impacting step, is limited to about a 6 to 12 inches size range. After magnetic separation, where only the magnetic metal and magnetic slags are present in the magnetic portion of the process burden, it is then possible to separate-out the clean metal in a size range from 3 to 6 inches, by screening from the minus 3 inch magnetic slag.

It is assumed in the illustrated process or layout of Figure 13, that the steel plant does not desire metal under 3 inches in size for open hearth use, or fines under  $\frac{1}{4}$  of an inch in size for direct blast furnace charging. Thus, subsequent refining and concentration procedures for minus 3 inch magnetic material are employed to meet such conditions. As will be noted, only two Ball-Norton separators are shown as used (stations 134 and 140), in contrast to the three units employed in the final processing layouts of Figures 1c and 12. Also, the feed size ranges are slightly different in the layout of Figure 13. Magnetic rejections from a second separator of Figure 13 are shown screened, and only the  $\frac{1}{8}$  to  $\frac{1}{4}$  of an inch size portion of the burden is shown crushed and re-cycled. On the other hand, the minus  $\frac{1}{8}$  of an inch size rejects of the burden are shown conveyed to a disposal conveyor.

It will also be noted that in the layout of Figure 13, non-magnetic slag under 3 inches in size is shown separated into size portions, which are separately crushed in two roll crushers and re-cycled for magnetic separation.

of their thus-released magnetic particle content, down to minus  $\frac{3}{8}$  of an inch size before their final disposal.

More specifically, in the layout of Figure 13, a ball-drop pit area is designated as 105 and a storage hopper 106 with a vibrating feeder discharge such as is shown in Figure 3 is employed to provide a delivery of minus 12 inches size slags and metal (which is received through its grid or screen passes of 12 inch mesh size) to a longitudinal continuously-forwardly-moving conveyor 107. 10 The conveyor 107 is shown as delivering the burden to a roller screen station 108 (such as in Figures 6 and 6a) that may have a pass opening of about 3 inches to deliver the minus 3 inches size portion or content of the burden to a second longitudinal continuously-forwardly-moving belt conveyor 109. On the other hand, the portion or content of the burden of 3 to minus 12 inches in size consisting of magnetic and non-magnetic slags and metals, is shown as passing over the bed of station 108 for delivery to a transverse continuously-forwardly-moving side belt conveyor 110. The burden of conveyor 110 is shown subjected to rotary impacting or breaking up at station 111 (see the apparatus of Figure 4) to provide a burden containing 3 to minus 12 inches size clean metal, minus 6 inches size non-magnetic slags, and 25 minus 3 inches magnetic slags. The latter burden is shown carried to roller screen station 112 that has a 6 inches size mesh, by a transverse continuously moving side belt conveyor 110a.

At roller screen station 112, clean metal of a size 30 range of 6 to minus 12 inches is shown as passing over the screen table for delivery to transverse continuously-moving side belt conveyor 113, to longitudinal continuously-forwardly-moving belt conveyor 113a, and is carried by transverse, continuously-moving side belt conveyor 122 to clean metal collecting or delivery area (8). It may be noted that the burden from conveyor 113a is shown combined with 3 to minus 6 inches size clean metal that is being delivered by conveyor 122 from another portion of the system, to provide metal at area (8) 40 of a full size range of about 3 to minus 12 inches.

The burden of longitudinal forwardly-moving conveyor 109 is shown advanced to a rectangular magnet station 114 and over a magnet pulley at magnetic pulley station 115 (see typical magnet apparatus of Figure 9) to 45 separate-out magnetic slags of minus 3 inches size and magnetic metals of minus 6 inches size as a magnetic burden that is delivered to a transverse continuously-forwardly-moving side belt conveyor 116. The burden of conveyor 116 is shown received by a longitudinal continuously-moving belt conveyor 116a for delivery upon the bed of a roller screen station 121 (3 inches size mesh).

At station 121, the larger size portion of the burden of 50 3 to minus 6 inches clean metal is shown as passing over the roller screen or bed for delivery to a transverse continuously-moving side belt conveyor 122, and thence, to collecting area (8). On the other hand, the smaller or minus 3 inches size portion of the burden at station 121 that consists of magnetic slags and metals that pass through the screen bed, is shown delivered by transverse continuously-forwardly-moving side belt conveyor 123 to a vibrating screen station 124 (see for example vibrating screen apparatus of Figures 9 and 10).

At screen station 124, the larger size portion or content of the burden is shown passing over the screen bed ( $\frac{3}{4}$  of an inch mesh), and as carried by longitudinal continuously-moving belt conveyor 126 to a rotary impact crushing station 127. The smaller size portion of the burden of minus  $\frac{3}{4}$  inch magnetic slags and metal is shown delivered to a transverse continuously-forwardly-moving side belt conveyor 125 and to a longitudinal continuously-forwardly-moving belt conveyor 131.

At station 127, the burden is shown impacted to provide a resultant burden for delivery to transverse continuously-forwardly-moving belt conveyor 128. This

burden is shown as now consisting of minus 3 inches size magnetic metal and minus  $\frac{3}{4}$  of an inch size magnetic slags, and as delivered by conveyor 128 to a vibrating screen station 130 (shown as having a  $\frac{3}{4}$  of an inch size mesh). Station 130 is shown as separating the burden into two portions consisting of a larger size portion of  $\frac{3}{4}$  to minus 3 inches size clean metal that passes over the screen and is delivered to a transverse continuously-forwardly-moving side belt conveyor 132, and of a smaller size portion of minus  $\frac{3}{4}$  of an inch magnetic slags and metal that passes through the screen and is delivered to longitudinal continuously-forwardly-moving belt conveyor 131. It will be noted that the burden of conveyor 132 is shown combined with the burden of conveyor 138 to provide a composite burden of  $\frac{1}{4}$  to minus 3 inches size clean metal and high iron content magnetic slags for delivery to collection area (10).

The burden of longitudinal conveyor 131 is shown delivered forwardly to a vibrating screen station 133 ( $\frac{1}{4}$  of an inch mesh size) at which it is separated into two size portions or contents. The smaller size content of minus  $\frac{1}{4}$  of an inch magnetic slags and metal is shown as passing through the screen and as delivered to longitudinal continuously-forwardly-moving belt conveyor 139. The larger size of  $\frac{1}{4}$  to minus  $\frac{3}{4}$  of an inch is shown delivered to magnetic separation station 134 (see the apparatus of Figure 11), where clean metal and high iron content magnetic slags of a size range of  $\frac{1}{4}$  to minus  $\frac{3}{4}$  of an inch are shown segregated and delivered to a longitudinal continuously-moving belt conveyor 138 to combine with the content of side conveyor 132 for delivery to area (10). On the other hand, the magnetic slags and metal rejects of  $\frac{1}{4}$  to minus  $\frac{3}{4}$  of an inch size are shown discharged on a continuously-moving belt conveyor 135 and delivered to a roller crusher station 136 (see roll crusher of Figure 9). The crusher station 136 (of  $\frac{1}{4}$  inch pass size), as shown, provides minus  $\frac{1}{4}$  crushed rejects that are discharged upon transverse continuously-moving belt conveyor 137 to combine with rejects from conveyors 146 and 150. The resultant burden is thus re-cycled by being delivered upon longitudinal forwardly-moving conveyor 109.

The relatively non-magnetic portion of the burden of longitudinal conveyor 109 is shown carried from magnet separator stations 114 and 115 to a roller screen station 117 (shown of 3 inches mesh or pass size) at which a 3 to minus 6 inch size portion of the non-magnetic slag burden passes over the screen bed and is discharged upon a transverse continuously-moving side belt conveyor 118 for delivery to collecting or delivery area (9). The smaller size portion or content of the non-magnetic slag burden at station 117 of minus 3 inches size is shown as passing through the roller screen and discharging upon transverse continuously-forwardly-moving side belt conveyor 120 for delivery to a vibrating screen station 148 (shown as having a 1 inch size mesh screen). At station 148, the portion of the non-magnetic slag burden of minus 1 inch in size is shown as passing through the screen and as discharged upon longitudinal continuously-forwardly-moving belt conveyor 151, while the 1 to minus 3 inches size portion of the non-magnetic slag burden is shown delivered over the screen to a crusher station 149. Station 149 is shown provided with a 1 inch roll pass; it delivers now-crushed slag of minus 1 inch size to a longitudinal continuously-moving belt conveyor 150. The conveyor 150 which also receives burden from station 154 is shown as discharging its burden upon transverse belt conveyor 137 to combine with the burden from stations 136 and 145.

The burden of forwardly-moving belt conveyor 151 is shown delivered to a vibrating screen station 152, shown as having  $\frac{3}{4}$  of an inch size mesh. At screening station 152,  $\frac{3}{4}$  to minus 1 inch size portion of the non-magnetic burden is shown as passing over the screen and as crushed at roll crusher station 154 which, as illustrated, has a  $\frac{3}{4}$

inch roll pass, and delivers the now minus  $\frac{3}{8}$  of an inch of the non-magnetic slag burden to longitudinal continuously-moving belt conveyor 150 to combine with the burden from crusher station 149.

At screening station 152, the minus  $\frac{3}{8}$  inch size portion or content of the non-magnetic slag burden is shown as passing through the screen bed for discharge upon a longitudinal continuously-forwardly-moving belt conveyor 153 which delivers it to collecting or disposal area (12). As shown, this burden is combined with burden from side conveyor 144 to provide a burden consisting of minus  $\frac{3}{8}$  non-magnetic slags and minus  $\frac{1}{8}$  magnetic slag rejects at area (12).

At vibrating screen station 133, the portion or content of the burden consisting of minus  $\frac{1}{4}$  inch magnetic slags and metals is shown discharged upon longitudinal continuously-forwardly-moving belt conveyor 139 for delivery to magnetic separator station 140. The separator station 140 is shown as delivering the higher magnetic content of the burden, consisting of minus  $\frac{1}{4}$  inch magnetic particles and high iron content magnetic slags, to a side conveyor 141 for delivery to a collecting or delivery area (11). The lower magnetic slag rejects of minus  $\frac{1}{4}$  inch of station 140 are shown discharged upon transverse continuously-forwardly-moving side belt conveyor 142 and as delivered to a vibrating screen station 143.

At station 143, the portion or content of the burden of  $\frac{1}{4}$  to  $\frac{1}{8}$  of an inch size is shown as passing over the bed and as delivered to a roller crusher station 145. Station 145 (of a  $\frac{1}{8}$  inch pass size) crushes the burden to minus  $\frac{1}{8}$  of an inch size and delivers it to a longitudinal continuously-moving belt conveyor 146. The minus  $\frac{1}{8}$  inch rejected portion of the burden at station 143 is shown as passing through its screen and as being discharged upon transverse continuously-forwardly-moving side belt conveyor 144 to combine with the burden of conveyor 153.

Summarized briefly, the layout, system or procedure of Figure 13 illustrates how to process a burden of minus 12 inches size slags and metals to provide 3 to minus 12 inches size clean metal at area (8) that is suitable for open hearth charging, to provide 3 to minus 6 inches size non-magnetic slag at area (9) that is suitable in limited quantities as a lime substitute in a blast furnace charge, to provide  $\frac{1}{4}$  to minus 3 inches size clean metal and high iron content slags at area (10) that is suitable for blast furnace utilization, to provide minus  $\frac{1}{4}$  metal particles and high iron content magnetic slags at area (11) that is suitable for sintering plant operation and subsequent blast furnace utilization, and to provide minus  $\frac{3}{8}$  inch size non-magnetic slags and minus  $\frac{1}{8}$  inch magnetic slag rejects at area (12) for any suitable use.

The diagram or layout of Figure 13 thus further illustrates the scope and nature of my invention, as well as its important coordinated operating principles that fully meet a long-standing problem in the art, and particularly, from the standpoint of, for the first time, making possible a substantially full and complete recovery of the value content of metal bearing refuse and debris that may result from metal processing operations.

What I claim is:

1. A process for recovering substantially clean metal pieces of a selected size range from a burden comprising a mixture of materials such as are found in steel plant debris and which includes metal pieces and friable material, which comprises impacting the burden with sufficient force to break up the friable portion thereof to a maximum size which is below the minimum of the selected size range and to render substantially clean the metal pieces of the selected size range, and subjecting the impacted burden to a sizing operation to separate from it the substantially clean metal pieces of the selected size range.

2. A process for recovering substantially clean metal pieces of a selected size range from a burden comprising

a mixture of materials such as are found in steel plant debris and which includes metal pieces and friable material, which comprises separating the burden by a sizing operation into a larger piece size portion and a smaller piece size portion, impacting the larger piece size portion with sufficient force to break up the friable portion thereof to a maximum size which is below the minimum of the selected size range and to render substantially clean the metal pieces of the selected size range, and subjecting the impacted larger piece size portion to a sizing operation to separate from it the substantially clean metal pieces of the selected size range.

3. A process for recovering substantially clean metal pieces of a selected size range from a burden comprising a mixture of materials such as are found in steel plant debris and which includes metal pieces and friable material, which comprises impacting the burden with sufficient force to break up the friable portion thereof to a maximum size which is below the minimum of the selected size range and to render substantially clean the metal pieces of the selected size range, subjecting the impacted burden to a sizing operation to separate from it the substantially clean metal pieces of the selected size range, and subjecting the remainder of the burden after processing as described to magnetic separation.

4. A process for recovering substantially clean metal pieces of a selected size range from a burden comprising a mixture of materials such as are found in steel plant debris and which includes metal pieces and friable material, which comprises separating the burden by a sizing operation into a larger piece size portion and a smaller piece size portion, impacting the larger piece size portion with sufficient force to break up the friable portion thereof to a maximum size which is below the minimum of the selected size range and to render substantially clean the metal pieces of the selected size range, subjecting the impacted larger piece size portion to a sizing operation to separate from it the substantially clean metal pieces of the selected size range, and subjecting the remainder of the larger piece size portion after processing as described and said smaller piece size portion to magnetic separation.

5. A process for recovering substantially clean metal pieces in progressively smaller piece size ranges from a burden comprising a mixture of materials such as are found in steel plant debris and which includes metal pieces and friable materials, which comprises impacting the burden with sufficient force to break up the friable portion thereof to a maximum size which is below the minimum of a selected piece size range and to render substantially clean the metal pieces of the selected piece size range, subjecting the impacted burden to a sizing operation to separate from it the substantially clean metal pieces of the selected piece size range, and subjecting the material from which said metal pieces have been separated to the defined steps to provide burden of smaller size range and to separate therefrom metal pieces of smaller size range.

6. A process according to claim 5, wherein the remainder of the burden after processing as defined is subjected to magnetic separation.

7. A process for recovering substantially clean metal pieces in progressively smaller piece size ranges from a burden comprising a mixture of materials such as are found in steel plant debris and which includes metal pieces and friable materials, which comprises separating the burden by a sizing operation into a larger piece size portion and a smaller piece size portion, impacting the larger piece size portion with sufficient force to break up the friable portion thereof to a maximum size which is below the minimum of a selected piece size range and to render substantially clean the metal pieces of the selected piece size range, subjecting the impacted burden to a sizing operation to separate from it the substantially clean metal pieces of the selected piece size range, and

progressively subjecting said smaller piece size portion and the material from which said metal pieces have been separated to the defined steps to provide burden of smaller size range and to separate therefrom metal pieces of progressively smaller size range.

8. A process according to claim 7, wherein the remainder of the burden after processing as defined is subjected to magnetic separation.

9. A process for separating substantially clean magnetic metal pieces of a selected size range from friable magnetic material such as open hearth tap slag, which comprises impacting a burden containing the magnetic metal pieces and friable magnetic material with sufficient force to break up the friable magnetic material to a maximum size which is below the minimum of the selected size range and to render substantially clean the magnetic metal pieces of the selected size range, and subjecting the impacted burden to a sizing operation to separate the substantially clean magnetic metal pieces of the selected size range from the broken-up friable magnetic material.

10. A process for separating substantially clean magnetic metal pieces of a selected size range from friable magnetic material such as open hearth tap slag, which comprises separating by a sizing operation a burden containing the magnetic metal pieces and friable magnetic material into a larger piece size portion and a smaller piece size portion, impacting the larger piece size portion with sufficient force to break up the friable magnetic material to a maximum size which is below the minimum of the selected size range and to render substantially clean the magnetic metal pieces of the selected size range, and subjecting the impacted larger piece size portion to a sizing operation to separate the substantially clean magnetic metal pieces of the selected size range from the broken-up friable magnetic material.

11. A process for recovering magnetic metal, magnetic slags and magnetic oxides from a burden comprising a mixture of materials such as are found in steel plant debris, which comprises subjecting the burden to a high intensity magnetic field to separate the burden into magnetic and non-magnetic portions, magnetically treating the magnetic portion to provide from it a higher magnetic product and a lower magnetic part, breaking up the lower magnetic part to release magnetic particles therefrom, and subjecting the broken-up lower magnetic part to magnetic treatment to recover therefrom further magnetic particles.

12. A process for recovering magnetic metal, magnetic slags and magnetic oxides from a burden comprising a mixture of materials such as are found in steel plant debris, which comprises subjecting the burden to a high intensity magnetic field to separate the burden into magnetic and non-magnetic portions, dividing the magnetic portion into size range components, separately magnetically treating at least two of the size range components to provide from each size range component a higher magnetic product and a lower magnetic part, breaking up at least one of the lower magnetic parts to release magnetic particles therefrom, and subjecting the broken-up lower magnetic part to magnetic treatment to recover therefrom further magnetic particles.

13. A process for recovering magnetic metal, magnetic slags and magnetic oxides from a burden comprising a mixture of materials such as are found in steel plant debris, which comprises subjecting the burden to a high intensity magnetic field to separate the burden into magnetic and non-magnetic portions, impacting the magnetic portion with sufficient force to break up the friable content thereof to a maximum size which is effectively smaller than the maximum size of the metal pieces contained therein, subjecting the impacted magnetic portion to a sizing operation to separate from it the metal pieces of a size which is between the maximum size of the metal pieces and the maximum size of the broken-up friable

content, and subjecting the remainder of the impacted magnetic portion from which the metal pieces have been separated to magnetic treatment to recover magnetic particles therefrom.

14. A process for recovering magnetic metal, magnetic slags and magnetic oxides from a burden comprising a mixture of materials such as are found in steel plant debris, which comprises subjecting the burden to a high intensity magnetic field to separate the burden into magnetic and non-magnetic portions, size separating the magnetic portion into a larger piece size component and a smaller piece size component, impacting the larger piece size component with sufficient force to break up the friable portion thereof to a maximum size which is effectively smaller than the maximum size of the metal pieces contained therein, subjecting the impacted larger piece size component to a sizing operation to separate from it the metal pieces of a size which is between the maximum size of the metal pieces and the maximum size of the broken-up friable portion, and subjecting the remainder of the impacted larger piece size component from which the metal pieces have been separated and said smaller piece size component to magnetic treatment to recover magnetic particles therefrom.

15. A process for recovering magnetic metal, magnetic slags and magnetic oxides from a burden comprising a mixture of materials such as are found in steel plant debris, which comprises subjecting the burden to a high intensity magnetic field to separate the burden into magnetic and non-magnetic portions, size separating the magnetic portion into a larger piece size component and a smaller piece size component, impacting the larger piece size component with sufficient force to break up the friable portion thereof to a maximum size which is effectively smaller than the maximum size of the metal pieces contained therein, subjecting the impacted larger piece size component to a sizing operation to separate from it the metal pieces of a size which is between the maximum size of the metal pieces and the maximum size of the broken-up friable portion, size separating the remainder of the impacted larger piece size component from which the metal pieces have been separated and said smaller piece size component into size range components, separately magnetically treating at least two of the size range components to provide from each size range component a higher magnetic product and a lower magnetic part, breaking up at least one of the lower magnetic parts to release magnetic particles therefrom, and subjecting the broken-up lower magnetic part to magnetic treatment to recover therefrom further magnetic particles.

16. A method of recovering metal in the nature of iron and steel of sufficient purity for open hearth utilization from slag dump refuse containing refractory material, magnetic and non-magnetic malleable metal, mag-

netic or non-magnetic friable slag and magnetic ore and metal of large to small sizes that are held by slag which comprises, continuously moving a mass of the slag dump refuse while progressively subjecting it to a rotary hammer impaction of increased intensity and freeing metal of progressively smaller size from the slag, passing the mass being impacted through passageways of progressively smaller size that at least correspond to the size of the metal to be then removed, breaking up the friable portions of the mass into a size smaller than the size of the metal to be then removed, selectively removing the metal of progressively smaller sizes by-passed by the impacting passages by size-separating it from the friable portions of the mass, and during the processing, progressively magnetically separating lower and non-magnetic from higher magnetic materials of the mass.

#### References Cited in the file of this patent

#### UNITED STATES PATENTS

|    |           |              |                |
|----|-----------|--------------|----------------|
| 20 | 160,618   | Rudy         | Mar. 9, 1875   |
|    | 1,002,967 | Cox          | Sept. 12, 1911 |
|    | 1,339,300 | Swart et al. | May 4, 1920    |
|    | 1,431,444 | De Coursey   | Oct. 10, 1922  |
|    | 1,498,144 | Avery        | June 17, 1924  |
| 25 | 1,617,971 | Ullrich      | Feb. 15, 1927  |
|    | 1,958,351 | Shingshang   | May 8, 1934    |
|    | 1,981,415 | Kennedy      | Nov. 20, 1934  |
|    | 2,031,352 | Wilson       | Feb. 18, 1936  |
|    | 2,038,374 | Mansfield    | Apr. 21, 1936  |
| 30 | 2,047,345 | Weis         | July 14, 1936  |
|    | 2,110,851 | Symons       | Mar. 8, 1938   |
|    | 2,220,330 | Symons       | Dec. 24, 1940  |
|    | 2,264,204 | Heckett      | Nov. 25, 1941  |
|    | 2,292,852 | Werner       | Aug. 11, 1942  |
|    | 2,310,758 | Werner       | Feb. 9, 1943   |
| 35 | 2,352,712 | Heckett      | July 4, 1944   |
|    | 2,468,321 | Bland        | Apr. 26, 1949  |
|    | 2,470,889 | Drescher     | May 24, 1949   |
|    | 2,644,644 | West         | July 7, 1953   |
| 40 | 2,721,035 | Lankford     | Oct. 18, 1955  |
|    | 2,726,815 | Heckett      | Dec. 13, 1955  |
|    | 2,728,454 | Heckett      | Dec. 27, 1955  |
|    | 2,767,928 | Hanse        | Oct. 23, 1956  |
| 45 | 2,780,417 | Harris       | Feb. 5, 1957   |

#### FOREIGN PATENTS

|         |               |               |
|---------|---------------|---------------|
| 462,588 | Great Britain | Mar. 11, 1937 |
| 943,389 | Germany       | May 17, 1956  |

#### OTHER REFERENCES

Magnetic Separation in Ore Dressing, by W. H. Dennis, Mine and Quarry Engineering, September 19, 1944, pages 223-225.

UNITED STATES PATENT OFFICE  
CERTIFICATION OF CORRECTION

Patent No. 2,971,703

February 14, 1961

Frank E. Rath

It is hereby certified that error appears in the above numbered patent requiring correction and that the said Letters Patent should read as corrected below.

Column 15, lines 39 and 40, for "see Figure 16 and Figure 7" read -- see Figure 1b and Figure 7 --.

Signed and sealed this 27th day of June 1961.

(SEAL)  
Attest:

ERNEST W. SWIDER  
Attesting Officer

DAVID L. LADD  
Commissioner of Patents